



US005447830A

**United States Patent** [19]

Pawlak et al.

[11] **Patent Number:** 5,447,830[45] **Date of Patent:** Sep. 5, 1995[54] **3-ANILINO PYRAZOLONE MAGENTA COUPLERS AND PROCESS**

[75] Inventors: **John L. Pawlak; David S. Bailey**, both of Rochester; **William R. Schleigh**, Brockport; **Charles E. Romano**; **Paul B. Merkel**, both of Rochester; **Sundaram Krishnamurthy**, Penfield, all of N.Y.

[73] Assignee: **Eastman Kodak Company**, Rochester, N.Y.

[21] Appl. No.: **83,842**

[22] Filed: **Jun. 25, 1993**

**Related U.S. Application Data**

[63] Continuation-in-part of Ser. No. 872,576, Apr. 23, 1992, abandoned, which is a continuation-in-part of Ser. No. 689,436, Apr. 23, 1991, Pat. No. 5,298,368.

[51] **Int. Cl.**<sup>6</sup> ..... **G03C 7/384**

[52] **U.S. Cl.** ..... **430/504; 430/555**

[58] **Field of Search** ..... **430/555, 359, 504**

[56] **References Cited**

## U.S. PATENT DOCUMENTS

5,250,405 10/1993 Merkel et al. ..... 430/544  
5,256,528 10/1993 Merkel et al. ..... 430/555  
5,262,292 11/1993 Krishnamurthy ..... 430/555  
5,298,368 3/1994 Merkel et al. ..... 430/554

## FOREIGN PATENT DOCUMENTS

2-40649 2/1990 Japan .....  
2040648 2/1990 Japan ..... 430/555

*Primary Examiner*—Lee C. Wright  
*Attorney, Agent, or Firm*—Arthur E. Kluegel

[57] **ABSTRACT**

Magenta image-dye couplers provide photographic elements and processes having superior photographic properties. The couplers are 3-anilino pyrazolone couplers having an aryl thio coupling-off group. The substituents of the coupler are specified to obtain advantageous properties.

**14 Claims, No Drawings**

## 3-ANILINO PYRAZOLONE MAGENTA COUPLERS AND PROCESS

**CROSS REFERENCE TO RELATED  
APPLICATION**

This application is a continuation-in-part of U.S. Ser. No. 07/872,576 filed Apr. 23, 1992, now abandoned which is in turn a continuation-in-part of U.S. Ser. No. 07/689,436 which was filed on Apr. 23, 1991, U.S. Pat. No. 5,298,368. 10

## BACKGROUND OF THE INVENTION

This invention relates to 3-anilinopyrazolone magenta dye-forming couplers having a particular parent group and thio coupling-off group that enables improved photographic properties and to photographic materials and processes comprising such couplers.

In color photographic silver halide materials and processes so-called four equivalent 3-anilino pyrazolone couplers have provided magenta dye images having useful properties. Examples of such compounds are described in, for example, U.S. Pat. Nos. 3,907,571, 3,928,044, 3,935,015, 4,199,361 and 3,519,429. An example of one such pyrazolone coupler, described in, for example, U.S. Pat. No. 3,519,429 is herein designated as comparison coupler C-1 and is represented by the formula:

15 The presence of an alkoxy group in the ortho position on the phenylthio coupling-off group of coupler C-2 has provided advantageous properties. However, this coupler has not been entirely satisfactory due to formation of undesired stain in a color photographic silver halide 20 element upon exposure and processing and because it does not provide desired image-dye density upon rapid machine processing. The coupler C-2 does not achieve full dye density, especially when the exposed color photographic element is machine processed without 25 Lippman fine grain silver halide being present in the photographic element which can be used to effect complete conversion of the leuco-dye to image dye. It has been desirable to reduce or avoid the need for added Lippman fine grain silver halide without diminishing



This prior art coupler has a number of disadvantages. Since C-1 is a four-equivalent coupler, more silver halide and coupler must be used to obtain adequate dye yield, when compared to two-equivalent couplers. This increases the costs associated with this type of coupler. In addition, the dye dark stability is quite poor and the coupler itself causes substantial yellow stain in areas of minimum density, especially when kept under humid conditions. 55

In color photographic silver halide materials and processes, pyrazolone couplers comprising arylthio coupling-off groups have provided magenta dye images having useful properties. Examples of such compounds are described in, for example, U.S. Pat. No. 4,413,054, Japanese published patent application 60/057839, U.S. Pat. Nos. 4,876,182, 4,900,657 and 4,351,897. An example of such a pyrazolone coupler described in, for example, U.S. Pat. No. 4,413,054 is designated herein as comparison coupler C-2 and is represented by the formula:

dye density in the processed color photographic silver halide element. It is believed that the alkoxy substituent undesirably stabilizes the leuco-dye thus preventing the completion of the dye formation process during development. This leads to loss of expected density and unpredictable results due to post-development dye formation. The prior art coupler C-2 does not therefore meet the industry needs.

Another example of a pyrazolone coupler known to the art, described in U.S. Pat. No. 4,853,319, is designated herein as comparison coupler C-3 and is represented by the formula:



The presence of an acylamino group in the ortho position on the phenylthio coupling-off group of coupler C-3 has provided advantageous properties. This coupler does not require Lippman fine grain silver halide in order to obtain adequate dye density upon rapid machine processing. However, this type of coupler does suffer from unwanted gains in green density in unexposed areas upon standing in the dark. Another problem with couplers of this type is that in the presence of polyvalent cations such as calcium, the amount of dye formed from a given amount of exposure is reduced relative to a process with no polyvalent cations. In particular, increasing amounts of calcium ion in a seasoned process leads to unacceptable losses in dye yield with this type of coupler.

Another example of a pyrazolone coupler known to the art, described in U.S. Pat. No. 4,853,319 is designated herein as comparison coupler C-4 and is represented by the formula:



This coupler also does not require Lippman fine grain silver halide in order to obtain adequate dye density upon rapid machine processing. However, this type of coupler also gives reduced dye yields in the presence of polyvalent cations, in particular, calcium ion.

Another type of coupler that has been considered is one having a pentachloro- substitution on the N phenyl ring (U.S. Pat. No. 4,876,182). While such materials provide advantageous properties they are not preferred because rings containing more than 3 chloro substituents present laborious and costly administrative orders relative to disposal.

It has been desired to provide a new 3-anilinopyrazolone coupler having a phenylthio coupling-off group in a color photographic silver halide element and process which is capable of forming a magenta dye image of good stability, with high dye yield based on rapid machine processing, and with reduction or omission of

Lippman fine grain silver halide in the element. In addition, it has been desired to provide such a coupler which displays reduced sensitivity to polyvalent metal cations commonly found in photographic processes, specifically calcium ion. Also, it has been desired to provide such a coupler which displays excellent thermal stability in areas of no light exposure. Further, it has been desired to provide a new pyrazolone coupler which provides a magenta dye after photographic processing that has a hue suitable for optimal color reproduction and color saturation. The couplers disclosed in U.S. Pat. No. 4,853,319 that gave dyes with good hue for optimal color reproduction were generally unstable on keeping and formed undesirable stain in areas of minimum density. Finally, it has been desired to provide a new pyrazolone coupler that has high activity. High activity couplers allow for reduced material laydowns of the magenta coupler and silver halide, which in turn leads to reduced costs and improved optical quality.

#### SUMMARY OF THE INVENTION

It has now been found that the foregoing problems can be solved by using the materials and process of this invention. The photographic element of the invention contains a support bearing at least one silver halide emulsion layer having associated therewith a 5-pyrazolone photographic coupler represented by the formula:



wherein

a) substituents X<sub>1</sub>, X<sub>2</sub>, Y, G<sub>1</sub>, and G<sub>2</sub> are individually selected from the group of halogen, alkyl, alkoxy, aryloxy, acylamino, alkylthio, arylthio, sulfonamido, sulfamoyl, sulfamido, carbamoyl, diacylamino, alkoxy carbonyl, aryloxy carbonyl, alkoxy sulfonyl, aryloxy sulfonyl, alkyl sulfonyl, alkylsulfoxyl, arylsulfoxyl, arylsulfonyl, alkylsulfonyl, alkoxy carbonyl amino, ary-

- loxycarbonylamino, alkylureido, arylureido, acyloxy, nitro, cyano, trifluoromethyl and carboxy, and, in the case of  $X_1$ ,  $X_2$  and  $Y$ , hydrogen;
- b) a, b, and c are individually integers from 0 to 3 provided that "a" cannot be an integer which, combined with the selection of  $X_1$  and  $X_2$ , allows the number of chloride substituents on the ring containing  $G_1$  to exceed 3;
- c)  $R_1$  is selected from  $G_1$  and hydroxyl;
- d)  $Z$  is selected from carbamoyl, alkoxy sulfonyl, aryloxy sulfonyl, alkylsulfonyl, arylsulfonyl, alkoxy carbonyl, aryloxycarbonyl, sulfamoyl, acyloxy, nitro, cyano, and an amine group of the formula:



wherein  $R_2$  is selected from the group consisting of hydrogen, alkyl, alkenyl, aryl, acyl, and heterocyclic;

$A$  is carbon or sulfur, and  $d$  is 1 when  $A$  is carbon and 1 or 2 when  $A$  is sulfur;

$B$  is selected from alkyl, aryl, and heterocyclic groups bonded to  $A$  by an atom of oxygen, nitrogen, sulfur, or carbon of the group  $B$ , wherein, in the case of a carbon bond,  $B$  has the formula:



wherein  $R_3$ ,  $R_4$ , and  $R_5$  are individually selected from hydrogen, halogen, alkyl, aryl, heterocyclic group and  $W$ , wherein  $W$  is selected from  $-OR_6$ ,  $-SR_6$ , and  $-NR_7R_8$ , wherein  $R_6$  is selected from alkyl, aryl, and heterocyclic groups, and  $R_7$  and  $R_8$  are individually selected from hydrogen, alkyl, aryl, acyl, alkylsulfonyl, arylsulfonyl and heterocyclic group, provided that when  $A$  is carbon at least one of  $R_3$ ,  $R_4$ , and  $R_5$  is not hydrogen or alkyl and provided that two of  $R_3$ ,  $R_4$  and  $R_5$  may join to form an aliphatic, aromatic or heterocyclic ring; and

e) the sum of the sigma values for  $X_1$ ,  $X_2$ ,  $G_1$ ,  $G_2$ , and  $Y$  is at least 1.3.

#### DETAILED DESCRIPTION OF THE INVENTION

In a preferred pyrazolone coupler represented by the above formula,  
 $Z$  is represented by the formula:



where  $R_2$  is selected from hydrogen, alkyl, alkenyl, aryl, acyl, and heterocyclic,  
 where  $R_3$  is selected from  $W$ , aryl, and heterocyclic group;

$R_4$  and  $R_5$  are individually selected from  $W$ , hydrogen, halogen, alkyl, aryl, and heterocyclic group;

$W$  is selected from  $-OR_6$ ,  $-SR_6$ , and  $-NR_7R_8$ ;  
 $R_6$  is selected from alkyl, aryl, and heterocyclic group;

$R_7$  and  $R_8$  individually are selected from hydrogen, alkyl, aryl, acyl, alkylsulfonyl, arylsulfonyl and heterocyclic group.

$R_2$  and  $R_3$  optionally join to form an alicyclic or heterocyclic ring, and two of  $R_3$ ,  $R_4$  and  $R_5$  optionally join to form an alicyclic, aromatic, or heterocyclic ring (where, under such circumstances, the remaining substituent may be eliminated as a substituent and become a pi bond in the case of an aromatic compound or, in the case of a nonaromatic unsaturated aliphatic or heterocyclic ring may be a bond forming part of a double bond in the ring).

It is understood throughout this specification and claims that any reference to a substituent by the identification of a group containing a substitutable hydrogen (e.g. alkyl, amine, aryl, alkoxy, heterocyclic, etc.), unless otherwise specifically stated, shall encompass not only the substituent's unsubstituted form but also its form substituted with any substituents which do not negate the advantages of this invention. It is further intended that the organic substituents shall not exceed 30 carbon atoms and shall preferably not exceed 20 carbon atoms.

Among the compounds defined above, a particularly preferred pyrazolone coupler is represented by the above formula wherein  $Z$  is represented by the formula:

30



wherein  $R_2$  is as defined above;  
 $R_4$  and  $R_5$  are individually selected from  $W$ , hydrogen, halogen, alkyl, aryl, and heterocyclic group;

$W$  is selected from  $-OR_6$ ,  $-SR_6$ , and  $-NR_7R_8$ ;  
 $R_6$  is selected from alkyl, aryl, and heterocyclic group;

$R_7$  and  $R_8$  individually are selected from hydrogen, alkyl, aryl, acyl, alkylsulfonyl, arylsulfonyl and heterocyclic group;

$R_9$ ,  $R_{10}$ ,  $R_{11}$ ,  $R_{12}$  and  $R_{13}$  are individually selected from hydrogen, halogen, nitro, cyano, carboxy, aryl, alkyl, alkoxy, aryloxy, acylamino, sulfonamido, sulfamoyl, sulfamido, carbamoyl, diacylamino, aryloxycarbonyl, alkoxy carbonyl, alkoxy sulfonyl, aryloxysulfonyl, alkylsulfoxyl, arylsulfoxyl, alkylsulfonyl, arylsulfonyl, alkylthio, arylthio, alkoxy carbonylamino, alkylureido, arylureido, and acyl.

The parameters sigma and pi have well established values. The values for these constants can be easily found in the published literature (C. Hansch and A. J. Leo, in "Substituent Constants for Correlation Analysis in Chemistry and Biology", Wiley, New York, 1979; Albert J. Leo, in "Comprehensive Medicinal Chemistry", edited by C. Hansch, P. G. Sammes, and J. B. Taylor, Pergamon Press, New York, Volume 4, 1990).

60 65 "The Chemists' Companion", A. J. Gordon and R. A. Ford, John Wiley & Sons, New York, 1972 and "Progress in Physical Organic Chemistry", V. 13, R. W. Taft, Ed., John Wiley & Sons, New York.) Gener-

ally,  $\pi$  increases with increasing lipophilicity (of the ring substituent with hydrogen=zero) and sigma increases with increasing electron withdrawing power of the substituent with hydrogen=zero. In calculating the values of  $\pi$ , all of the components of a substituent must be considered. For sigma, only the atoms close to the ring have an electron withdrawing effect and remote atoms have no effect.

The pyrazolone coupler can be a monomeric, dimeric, trimeric, oligomeric or polymeric coupler, wherein the coupler moiety can be attached to the polymeric backbone via a substituent on the pyrazolone nucleus, or a substituent of the coupling-off group.

Examples of  $G_1$ ,  $G_2$ ,  $X_1$ ,  $X_2$ ,  $Y$ ,  $R_1$ ,  $R_9$ ,  $R_{10}$ ,  $R_{11}$ ,  $R_{12}$  and  $R_{13}$  include halogen, such as chlorine, bromine or fluorine; alkyl, including straight or branched chain alkyl, such as alkyl containing 1 to 30 carbon atoms, for example methyl, trifluoromethyl, ethyl, t-butyl, and tetradecyl; alkoxy, such as alkoxy containing 1 to 30 carbon atoms, for example methoxy, ethoxy, 2-ethylhexyloxy and tetradecyloxy; acylamino, such as acetamido, benzamido, butyramido, tetradecanamido,  $\alpha$ -(2,4-di-t-pentylphenoxy)-acetamido,  $\alpha$ -(2,4-di-t-pentylphenoxy)butyramido,  $\alpha$ -(3-pentadecylphenoxy)hexanamido,  $\alpha$ -(4-hydroxy-3-t-butylphenoxy)tetradecanamido, 2-oxo-pyrrolidin-1-yl, 2-oxo-5-tetradecyl-pyrrolin-1-yl, N-methyltetradecanamido, and t-butylcarbonamido; sulfonamido, such as methanesulfonamido, benzenesulfonamido, p-toluenesulfonamido, p-dodecylbenzenesulfonamido, N-methyltetradecylsulfonamido, and hexadecanesulfonamido; sulfamoyl, such as N-methylsulfamoyl, N-hexadecylsulfamoyl, N, N-dimethylsulfamoyl; N-[3-(dodecyloxy)propyl]sulfamoyl, N-[4-(2,4-di-t-pentylphenoxy)butyl]sulfamoyl, N-methyl-N-tetradecylsulfamoyl, and N-dodecylsulfamoyl; sulfamido, such as N-methylsulfamido and N-octadecylsulfamido; carbamoyl, such as N-methylcarbamoyl, N-octadecylcarbamoyl, N-[4-(2,4-di-t-pentylphenoxy)butyl]carbamoyl, N-methyl-N-tetradecylcarbamoyl, and N,N-diethylcarbamoyl; diacylamino, such as N-succinimido, N-phthalimido, 2,5-dioxo-1-oxazolidinyl, 3-dodecyl-2,5-dioxo-1-imidazolyl, and N-acetyl-N-dodecylamino; aryloxycarbonyl, such as phenoxy carbonyl and p-dodecyloxyphenoxy carbonyl; alkoxy carbonyl, such as alkoxy carbonyl containing 2 to 30 carbon atoms, for example methoxycarbonyl, tetradecyloxycarbonyl, ethoxycarbonyl, benzyloxycarbonyl, and dodecyloxycarbonyl; alkoxy sulfonyl, such as alkoxy sulfonyl containing 1 to 30 carbon atoms, for example methoxysulfonyl, octyloxysulfonyl, tetradecyloxysulfonyl, and 2-ethylhexyloxysulfonyl; aryloxysulfonyl, such as phenoxy sulfonyl, 2,4-di-t-pentylphenoxy sulfonyl. Alkanesulfonyl, such as alkanesulfonyl containing 1 to 30 carbon atoms, for example methanesulfonyl, octanesulfonyl, 2-ethylhexanesulfonyl, and hexadecanesulfonyl; arenesulfonyl, such as benzenesulfonyl, 4-nonylbenzenesulfonyl, and p-toluenesulfonyl; alkylthio, such as alkylthio containing 1 to 22 carbon atoms, for example ethylthio, octylthio, benzylthio, tetradecylthio, and 2-(2,4-di-t-pentylphenoxy)ethylthio; arylthio, such as phenylthio and p-tolylthio; alkoxy carbonyl amino, such as ethoxycarbonyl amino, benzyloxycarbonyl amino, and hexadecyloxycarbonyl amino; alkylureido, such as N-methylureido, N, N-dimethylureido, N-methyl-N-dodecylureido, N-hexadecylureido, N, N-dioc-tadecylureido, and N, N-diethyl-N'-ethyl-ureido; acyloxy, such as acyloxy, benzyloxy, oc-

tadecanoxyloxy, p-dodecanamido benzoyloxy, and cyclohexanecarbonyloxy; nitro; cyano and carboxy ( $-COOH$ ) and, except for  $G_1$ ,  $G_2$  and  $R_1$ , hydrogen.

Examples of  $Y$  as alkoxy include methoxy, ethoxy, 5 propoxy, butoxy, 2-methoxyethoxy, sec-butoxy, hexyloxy, 2-ethylhexyloxy, 2-(2,4-di-t-pentylphenoxy) ethoxy, and 2-dodecyloxyethoxy. Examples of  $Y$  as aryloxy include phenoxy,  $\alpha$ - $\beta$ -naphthoxy, and 4-tolyloxy.

The term "coupler" herein refers to the entire compound, including the coupler moiety and the coupling-off group. The term "coupler moiety" "(COUP)" or parent refers to that portion of the compound other than the coupling-off group.

The coupler moiety (COUP) can be any 3-anilinopyrazolone coupler moiety useful in the photographic art to form a color reaction product particularly a magenta dye, with oxidized color developing agent provided the substituents meet the requirements above described. Useful pyrazolone coupler moieties are described in, for example, U.S. Pat. Nos. 4,413,054; 4,853,319; 4,443,536; 4,199,361; 4,351,897; 4,385,111; Japanese Published Patent Application 60/170854; U.S. Pat. Nos. 3,419,391; 3,311,476; 3,519,429; 3,152,896; 2,311,082; and 2,343,703; the disclosures of which are incorporated herein by reference. The coupling-off group, if any, on the pyrazolone coupler moiety described in these patents or patent applications can be replaced by a coupling-off group according to the invention. The pyrazolone coupler according to the invention can be in a photographic element in combination with other magenta couplers known or used in the photographic art, such as in combination with at least one of the pyrazolone couplers described in these patents or published patent applications of the invention. The COUP portion of the couplers can be obtained as is known to the art. For example, syntheses of COUP moieties are described in Item 16736 in Research Disclosure, Mar. 1978; U.K. Patent Specification 1,530,272; U.S. Pat. Nos. 3,907,571; and 3,928,044.

In a particular embodiment, the coupling-off group contains a  $Z$  substituent which is a carbonamido group of the formula:



where the carbon connecting  $\text{R}_3$ ,  $\text{R}_4$ , and  $\text{R}_5$  to the carbonyl carbon is nonchiral. Typically, two or more of the  $\text{R}_3$ ,  $\text{R}_4$ , and  $\text{R}_5$  substituents may be hydrogen or methyl, for example. It is also possible that two of the substituents may be joined to form a ring which is nonchiral if the ring is symmetric about the central carbon. It has been found suitable to employ as one of the substituents an aryloxy compound ( $-\text{OR}_6$ ) and particularly suitable to employ an alkylaryloxy containing one or more alkyl substituents where the alkyl substituents are less than 30 carbon atoms, and typically less than 24 carbon atoms. It has also been found desirable under such circumstances to employ a sulfone as an electron-withdrawing group on the coupler parent, normally on the anilino ring.

Illustrative couplers include:



M-1



M-2



M-3



M-4



M-5



M-6



M-7

11

5,447,830



12

-continued

M-8



M-9



M-10



M-11



M-12



M-13



M-14



M-15

-continued



M-16



M-17



M-18



M-19



M-20



M-21



M-22

-continued



Q herein represents a coupling-off group according to the invention. Examples of Z include sulfamoyl, such as N-methylsulfamoyl, N-hexadecylsulfamoyl, N, N-dimethylsulfamoyl; N-[3-(dodecyloxy)propyl]sulfamoyl, N-[2,4-di-t-pentylphenoxy]butyl-sulfamoyl, N-methyl-N-tetradecylsulfamoyl; and N-dodecylsulfamoyl; carbamoyl, such as N-methylcarbamoyl, N-octadecylcarbamoyl, N-[4-(2,4-di-t-pentylphenoxy)butyl]carbamoyl, N-methyl-N-tetradecylcarbamoyl, and N,N-diethylcarbamoyl; aryloxycarbonyl, such as phenoxy carbonyl and p-dodecyloxyphenoxy carbonyl; alkoxy carbonyl, such as alkoxy carbonyl containing 2 to 30 carbon atoms, for example methoxycarbonyl, tetradecyloxycarbonyl, ethoxycarbonyl, benzyloxycarbonyl, and dodecyloxycarbonyl; alkoxy sulfonyl, such as alkoxy sulfonyl containing 1 to 30 carbon atoms, for example methoxysulfonyl, octyloxysulfonyl, tetradecyloxysulfonyl, and 2-ethylhexyloxysulfonyl; aryloxysulfonyl, such as phenoxy sulfonyl, 2,4-di-t-pentylphenoxy sulfonyl, alkylsulfonyl, such as alkylsulfonyl containing 1 to 30 carbon atoms, for example methanesulfonyl, octanesulfonyl, 2-ethylhexanesulfonyl, and hexadecanesulfonyl; arylsulfonyl, such as benzene-sulfonyl, 4-nonylbenzenesulfonyl, and p-toluenesulfonyl; acyloxy; such as acetoxy, benzoyloxy, octadecanoyloxy, p-dodecanamido-benzoyloxy, and cyclohexanecarbonyloxy; nitro; cyano, acyloxy and specified carbonamido and sulfonamido compounds. Illustrative coupling-off groups (Q) are as follows:

M-23



Q-4



Q-5



Q-6



Q-7



Q-8



Q-9



Q-10

65

5,447,830

**17**

-continued

**18**

-continued

Q-11 5 Q-19



Q-12 10 Q-20



Q-13 20 Q-21



Q-14 30 Q-22



Q-15 35 Q-23



Q-16 40 Q-24



Q-17 45 Q-25



Q-18 50 Q-26



Q-19 55 Q-27





-continued



The pyrazolone couplers preferably comprise a ballast group. The ballast group can be any ballast known in the photographic art. The ballast is typically one that does not adversely affect reactivity, stability and other desired properties of the coupler of the invention and does not adversely affect the stability, hue and other desired properties of the dye formed from the coupler. Illustrative useful ballast groups are described in the following examples.

Couplers of this invention can be prepared by reacting the parent 4-equivalent coupler containing no coupling-off group with the aryl disulfide of the coupling-off group according to the invention. This is a simple method and does not involve multiple complicated synthesis steps. The reaction is typically carried out in a solvent, such as dimethylformamide or pyridine.

The couplers according to the invention can be prepared by the following illustrative synthetic scheme, where COUP represents the coupler moiety having the coupling-off group attached at its coupling position:



wherein COUP is the coupler moiety and R<sub>1</sub>, R<sub>2</sub>, R<sub>4</sub>, R<sub>5</sub>, and R<sub>9</sub> through R<sub>13</sub> are as defined.

The following examples illustrate the preparation of couplers of this invention.

**Synthesis Example A: Synthesis of the Coupling Off Group.**

**Synthesis of o-Aminophenyl Disulfide**



A 1-L flask equipped with a magnetic stirring bar and a reflux condenser was charged with o-aminobenzenethiol (200 g, 1.6 moles) and dimethylsulfoxide (500 mL). The well stirred mixture was gently heated ( $\sim 50^\circ \text{C}$ .); the reaction was monitored to completion (2.5 hr, TLC, ligroin 950:EtOAc, 2:1). The mixture was poured into crushed ice. The product, o-aminophenyl disulfide was collected as a greenish yellow solid (169 g, 85% yield). This was further purified by recrystallization from hot methanol to furnish pale yellow solid, mp 88°-89° C.; HPLC=99%.

**Synthesis of o-(2,4-di-tert-Pentylphenoxy)butyramidophenyl Disulfide**



25 A 1-L round-bottom flask, equipped with a magnetic stirring bar, was charged with 2-(2,4-di-tert-pentylphenoxy)butyric acid (68.8 g, 210 mmol) and 250 mL of dichloromethane. To this well stirred solution of the acid, maintained ca. 25° C. (water-bath), oxalyl chloride (28.5 g, 220 mmol) was added through the dropping funnel. The resulting mixture was cooled (0° C., ice-bath) and N,N-dimethylformamide (DMF, 0.2 mL) was added as the catalyst. The reaction was stirred at 25° C. to completion (monitored by esterification with methanol and TLC analysis in ligroin 950:EtOAc 2:1). Removal of solvents on a rotary evaporator furnished the desired acid chloride as a pale yellow viscous liquid.



50 The acid chloride thus synthesized was dissolved in tetrahydrofuran (THF, 100 mL) and added dropwise through a pressure equalized addition funnel to a 1-L flask containing magnetically stirred solution of o-aminophenyl disulfide (24.8 g, 100 mmol) in 200 mL of THF and 75 mL of pyridine. The reaction was monitored to completion by TLC (20 min). The mixture was poured into crushed ice and the precipitate was collected; the crude product o-(2,4-di-tert-pentylphenoxy)butyramidophenyl disulfide, was further purified by recrystallization from a mixture of acetonitrile and pro-

pionitrile to afford 35 g (41% yield) of the desired product. HPLC: 99.1%. Anal Calcd for  $C_{52}H_{72}O_4N_2S_2$ : C, 73.2; H, 8.5; N, 3.3; S, 7.5. Found: C, 73.2; H, 8.3; N, 2.9; S, 7.0. The  $^1H$  NMR spectrum ( $CDCl_3$ , 300 MHz) was consistent with the structure.

Synthesis Example B: Synthesis of Coupler 1-15.



A 250 mL flask equipped with a magnetic stirring bar and a pressure equalizing addition funnel was charged with *o*-(2,4-di-*tert*-pentylphenoxy)butyramidophenyl disulfide (14.6 g, 16.4 mmol), pyrazolone coupler (MW 636.5, 20.0 g, 31.4 mmol), and DMF (100 mL). To this well stirred slurry, bromine (0.81 mL, 15.8 mmol) dissolved in DMF (15 mL) was added dropwise through an addition funnel. The resulting mixture was heated to  $\sim 60^\circ C$ , and maintained at that temperature. After 1 h, TLC analysis showed unreacted coupler, so additional  $Br_2$  (0.05 mL, 1.0 mmol) was added. After another 0.5 h, the mixture was poured into crushed ice and the resulting product was filtered to afford the desired coupler in quantitative yield. This was further purified by flash chromatography on silica gel [EtOAc/Ligroin (1:10)–2 L, (1:5)–6 L, (1:3)–2 L, (1:2)–2 L, (1:1)–4 L, (3:2)–2 L; 1 L fractions, 10  $\times$  15 cm column]. Concentration of fractions 8–17 gave 31.3 g of M-11 (94% yield). Alternatively, the crude mixture could be recrystallized from EtOAc/Ligroin ( $\sim 1:10$ ) to afford pure M-11.

Synthesis Example C: Synthesis of Coupler 1-28



Sulphydryl chloride (5.1 g, 37.5 mmol) was added to a solution of the disulfide (*o*-(2,4-Di-*tert*-pentylphenoxy)butyramidophenyl disulfide, 32.0 g, 37.5 mmol), in dichloromethane (150 mL). After 1.75 hr, the volatiles were removed by rotary evaporation below  $40^\circ C$ . A solution of the pyrazolone coupler (MW 621, 45.0 g, 72.5 mmol) in DMF (200 mL) was added rapidly to the oil. After stirring at room temperature for 51 hr, the mixture was poured slowly into 3N HCl (1500 mL). The sticky solid was collected by filtration and the residue was dissolved in ethyl acetate (700 mL). The organic solution was washed with water ( $2 \times 150$  mL), dried and evaporated under reduced pressure. The crude material was purified by column chromatography on silica gel [EtOAc/Ligroin (1:2)]. The resulting oil was dissolved in acetic acid (100 mL) and precipitated by addition to water (4000 mL). The solid was collected by filtration to give I-30 as a white solid (49.0 g, 65%).

Synthesis Example D: Synthesis of Coupler I-31

Synthesis of Coupling-off Group Q-8.

Synthesis of Methyl (3-Pentadecylphenoxy) acetate



A 1-L three necked flask, equipped with a mechanical stirrer, pressure equalizing addition funnel, and a reflux condenser was charged with 1-L of reagent grade acetone, 3-pentadecylphenol (100 g, 0.328 mol), and anhydrous potassium carbonate (82 g, 0.6 mol). To this well stirred solution, methyl bromoacetate (69 g, 0.7 mol) was added through the addition funnel. The resulting

mixture was vigorously stirred and heated to gentle reflux over a heating mantle. The reaction was monitored by TLC (5:1 ligroin 950 and EtOAc). The reac-

Synthesis of 2-(3-Pentadecylphenoxyacetamido)phenyl Disulfide, Q-8



tion was continued overnight to completion and then cooled to room temperature. Potassium carbonate was filtered. After a few minutes of standing, the product precipitated. The volatiles were removed on a rotary evaporator to afford a beige solid. This was further purified by recrystallization from hot methanol to give 108 g (88% yield) of the desired ester, mp 44°C.

#### Synthesis of (3-Pentadecylphenoxy)acetic Acid



A 2-L round bottom flask equipped with a magnetic stirring bar and a reflux condenser was charged with potassium hydroxide (28 g, 0.5 mol) and methanol (1-L). To this vigorously stirred mixture, methyl (3-pentadecylphenoxy)acetate (93 g, 0.247 mol) was added and the resulting slurry was brought to a gentle reflux (2 hr). The ester was not completely soluble. The reaction was monitored by TLC. The hydrolysis was complete in 2 hr. The mixture was cooled and poured into crushed ice-water-hydrochloric acid mixture to precipitate the acid as white solid. The acid was dried and further purified by trituration from hot methanol to afford 82 g (92% yield) of the acid, mp 96°C.

25 A 500-mL flask, equipped with a magnetic stirring bar was charged with 3-pentadecylphenoxyacetic acid (27.1 g, 75 mmoles) and dichloromethane (200 ml). To this well stirred slurry, oxalyl chloride (10.2 g, 80 mmoles) was added dropwise through an addition funnel. N,N-Dimethylformamide (0.5 ml) was added to serve as the catalyst.

26 A vigorous gas evolution was observed and the solution became clear in 45 min. The reaction was complete (methanolysis of an aliquot and analysis by TLC in 2:1 ligroin 950: EtOAc) in 2 hr. Removal of volatile solvents on a rotary evaporator furnished the desired acid chloride (28.6 g, 100% yield) as a viscous oil.

30 A 1-L flask equipped with a magnetic stirring bar and a pressure equalizing dropping funnel was charged with o-aminophenyl disulfide (8 g, 32 mmoles), tetrahydrofuran (THF, 35 ml), and pyridine (35 ml). To this well stirred solution, previously synthesized acid chloride dissolved in dry THF was added through the addition funnel. The mixture was well stirred and monitored by TLC (ligroin 950:EtOAc, 5:1). The reaction was complete in 1 hr. The mixture was poured into crushed ice-water mixture, stirred well, and the resulting cream colored solid filtered and dried (30 g, ~100% yield). The crude product was further purified by recrystallization from 3:1 mixture of hot n-butyronitrile and acetonitrile to furnish 3-pentadecylphenoxyphenyl disulfide (26 g, 87%) as pale yellow crystals, mp 89°–90°C. Calculated for  $\text{C}_{58}\text{H}_{84}\text{N}_2\text{O}_4\text{S}_2$ : C, 74.31; H, 9.03; N, 2.99; S, 6.84. Found: C, 74.56; H, 8.91; N, 2.92; S, 7.18.

#### Synthesis of Coupler I-31



-continued



I-31

A 500-mL flask equipped with a magnetic stirring bar and a reflux condenser connected to a mineral oil bubbler was charged with the 4-equivalent pyrazolone magenta coupler (M-20, 9.6 g, 15.5 mmoles, FEW 621) and 3-pentadecylphenoxyphenyl disulfide (9.8 g, 8.5 mmoles), and DMF (70 ml). The disulfide did not dissolve in DMF completely. To this, bromine (1.5 g, 9.35 mmoles) dissolved in DMF (6 ml) was added. The resulting mixture was heated (60°–70° C.) and the reaction monitored by TLC to completion (2 hr). TLC analysis revealed the reaction to be clean essentially affording a single product. The mixture was cooled to room temperature and poured into a mixture of crushed ice and water. The coupler was extracted with ethyl acetate and the removal of volatile provided a red oil. Addition of a 1:3 mixture of n-butyronitrile and acetonitrile fol-

lowed by warming and cooling precipitated the coupler as a creamy solid (17 g, 100%, HPLC 97%). This was further recrystallized from hot butyronitrile (13.7 g, 78% yield), mp 98°–99° C. Calculated for  $C_{56}H_{74}Cl_4N_4O_5S_2$ : C, 61.75; H, 6.84; N, 5.14; Cl, 13.02; S, 5.88. Found: C, 61.69; H, 6.78; N, 5.24; Cl, 13.0; S, 6.37. FDMS (M<sup>+</sup>): 1079.

The purity of the two-equivalent couplers synthesized was checked by (a) TLC in two or three different solvent systems of different polarity, (b) HPLC, (c) 300 MHz FT-NMR and (d) elemental analyses (C, H, N, Cl, S); some samples were also subjected to mass spectral analysis.

The following structures are included for comparative purposes:



CM-1



CM-2



CM-3

29

5,447,830

30

-continued



CM-4



CM-5



CM-6



CQ-1



CQ-2



CQ-3



CQ-4



CQ-5



CQ-6

-continued

CQ-7



The following compounds were prepared by this 10 general method:

TABLE I

| Coupler | HPLC<br>Purity <sup>c</sup> | Elemental Analysis |              |            |            |              | mp, °C.    | Type      | COUP/Q     |          |
|---------|-----------------------------|--------------------|--------------|------------|------------|--------------|------------|-----------|------------|----------|
|         |                             | C                  | H            | N          | Cl         | S            |            |           |            |          |
| C-1     | na                          | calc.<br>found     | na           |            |            |              | 179-180    | Check     | CM-1/Q = H |          |
| C-2     | na                          | calc.<br>found     | na           |            |            |              | 165-167    | Check     | CM-2/CQ-1  |          |
| C-3     | na                          | calc.<br>found     | na           |            |            |              | 129-133    | Check     | CM-2/CQ-2  |          |
| C-4     | 99.4                        | calc.<br>found     | na           |            |            |              | 86-90      | Check     | CM-3/Q-22  |          |
| C-5     | 99.6                        | calc.<br>found     | 63.5<br>63.8 | 6.9<br>6.7 | 6.7<br>6.5 | 13.6<br>13.3 | 3.1<br>3.2 | 201-203   | Check      | CM-2/Q-1 |
| C-6     | 95.5                        | calc.<br>found     | na           |            |            |              | glass      | Check     | CM-4/CQ-2  |          |
| C-7     | 97.0                        | calc.<br>found     | na           |            |            |              | glass      | Check     | CM-5/Q-1   |          |
| C-8     | na                          | calc.<br>found     | na           |            |            |              | na         | Check     | M-11/CQ-2  |          |
| C-9     | na                          | calc.<br>found     | 54.1<br>53.7 | 5.6<br>5.5 | 8.3<br>8.2 |              | 98         | Check     | M-11/CQ-3  |          |
| C-10    | na                          | calc.<br>found     | 58.2<br>58.5 | 6.7<br>6.7 | 7.2<br>7.0 |              | 112        | Check     | M-11/CQ-4  |          |
| C-11    | na                          | calc.<br>found     | 54.1<br>54.0 | 5.6<br>5.5 | 8.3<br>8.2 |              | 100        | Check     | M-11/CQ-5  |          |
| C-12    | 88.1                        | calc.<br>found     | na           |            |            |              | glass      | Check     | M-11/CQ-6  |          |
| C-13    | na                          | calc.<br>found     | na           |            |            |              | na         | Check     | CM-2/Q-29  |          |
| C-14    | na                          | calc.<br>found     | na           |            |            |              | 163        | Check     | CM-6/CQ-7  |          |
| I-1     | 95.8                        | calc.<br>found     | na           |            |            |              | glass      | Invention | M-1/Q-1    |          |
| I-2     | 87.2                        | calc.<br>found     | na           |            |            |              | glass      | Invention | M-1/Q-4    |          |
| I-3     | 96.8                        | calc.<br>found     | na           |            |            |              | glass      | Invention | M-1/Q-6    |          |
| I-4     | 93.9                        | calc.<br>found     | na           |            |            |              | glass      | Invention | M-1/Q-2    |          |
| I-5     | 97.9                        | calc.<br>found     | na           |            |            |              | glass      | Invention | M-2/Q-1    |          |
| I-6     | 99.9                        | calc.<br>found     | na           |            |            |              | glass      | Invention | M-3/Q-1    |          |
| I-7     | 99.7                        | calc.<br>found     | na           |            |            |              | glass      | Invention | M-4/Q-1    |          |
| I-8     | na                          | calc.<br>found     | 58.6<br>56.8 | 5.9<br>5.6 | 7.0<br>7.1 | 14.1<br>13.6 | glass      | Invention | M-5/Q-1    |          |
| I-9     | na                          | calc.<br>found     | 58.5<br>58.5 | 6.1<br>5.9 | 7.0<br>6.9 |              | 196-199    | Invention | M-6/Q-1    |          |
| I-10    | 99.7                        | calc.<br>found     | na           |            |            |              | glass      | Invention | M-7/Q-1    |          |
| I-11    | 93.0                        | calc.<br>found     | na           |            |            |              | glass      | Invention | M-7/Q-15   |          |
| I-12    | na                          | calc.<br>found     | 58.6<br>57.3 | 5.9<br>5.7 | 7.0<br>7.0 | 14.1<br>14.6 | glass      | Invention | M-8/Q-1    |          |
| I-13    | 99.8                        | calc.<br>found     | na           |            |            |              | glass      | Invention | M-9/Q-1    |          |
| I-14    | 86.6                        | calc.<br>found     | na           |            |            |              | glass      | Invention | M-10/Q-1   |          |
| I-15    | 96.9                        | calc.<br>found     | na           |            |            |              | glass      | Invention | M-11/Q-1   |          |
| I-16    | 96.4                        | calc.<br>found     | na           |            |            |              | glass      | Invention | M-11/Q-4   |          |
| I-17    | 94.8                        | calc.<br>found     | na           |            |            |              | glass      | Invention | M-11/Q-6   |          |
| I-18    | na                          | calc.<br>found     | 59.2<br>59.8 | 6.3<br>6.3 | 6.8<br>6.8 |              | 107        | Invention | M-11/Q-9   |          |

TABLE I-continued

| Coupler | HPLC<br>Purity <sup>c</sup> | Summary of Batho-shifted 3-Anilino 4-(Arylthio)<br>Pyrazolone Couplers <sup>a, b</sup> |              |            |            |              |            |           |           |          |
|---------|-----------------------------|----------------------------------------------------------------------------------------|--------------|------------|------------|--------------|------------|-----------|-----------|----------|
|         |                             | Elemental Analysis                                                                     |              |            | mp, °C.    | Type         | COUP/Q     |           |           |          |
|         |                             | C                                                                                      | H            | N          | Cl         | S            |            |           |           |          |
| I-19    | 99.6                        | calc.<br>found                                                                         | na           |            |            | glass        | Invention  | M-11/Q-2  |           |          |
| I-20    | 72.0                        | calc.<br>found                                                                         |              |            |            | glass        | Invention  | M-11/Q-15 |           |          |
| I-21    | 98.5                        | calc.<br>found                                                                         | na           |            |            | glass        | Invention  | M-11/Q-21 |           |          |
| I-22    | 96.0                        | calc.<br>found                                                                         | na           |            |            | glass        | Invention  | M-11/Q-22 |           |          |
| I-23    | 97.4                        | calc.<br>found                                                                         | na           |            |            | glass        | Invention  | M-13/Q-1  |           |          |
| I-24    | 97.6                        | calc.<br>found                                                                         | na           |            |            | glass        | Invention  | M-15/Q-1  |           |          |
| I-25    | na                          | calc.<br>found                                                                         | 58.1<br>57.7 | 6.3<br>6.2 | 6.4<br>6.2 | glass        | Invention  | M-17/Q-1  |           |          |
| I-26    | na                          | calc.<br>found                                                                         | 55.7<br>56.2 | 4.8<br>5.0 | 6.3<br>6.1 | glass        | Invention  | M-18/Q-1  |           |          |
| I-27    | 92.6                        | calc.<br>found                                                                         | na           |            |            | glass        | Invention  | M-19/Q-1  |           |          |
| I-28    | 94.3                        | calc.<br>found                                                                         | 60.8<br>60.5 | 6.6<br>6.5 | 5.3<br>5.2 | 13.5<br>13.3 | 6.1<br>5.9 | glass     | Invention | M-20/Q-1 |
| I-29    |                             | calc.<br>found                                                                         | na           |            |            | glass        | Invention  | M-1/Q-29  |           |          |
| I-30    |                             | calc.<br>found                                                                         | na           |            |            | glass        | Invention  | M-20/Q-29 |           |          |
| I-31    |                             | calc.<br>found                                                                         | 61.8<br>61.6 | 6.8<br>6.8 | 5.1<br>5.2 | 13.0<br>13.0 | 5.9<br>6.4 | 98-99     | Invention | M-20/Q-8 |
| I-32    |                             |                                                                                        |              |            |            | 134-126      | Invention  | M-20/Q-47 |           |          |
| I-33    |                             | calc.<br>found                                                                         | 59.4<br>58.6 | 6.1<br>6.2 | 5.7<br>5.5 | 14.3<br>14.0 | 109-111    | Invention | M-20/Q-11 |          |
| I-34    |                             |                                                                                        |              |            |            | 258          | Invention  | M-20/Q-48 |           |          |
| I-35    | 94.9                        |                                                                                        |              |            |            | glass        | Invention  | M-20/Q-2  |           |          |

<sup>a</sup>All new couplers exhibited satisfactory <sup>1</sup>H NMR (FT-300 MHz).<sup>b</sup>Couplers were homogeneous in solvent systems of different polarity.<sup>c</sup>The values represent minimum since some decomposition is observed with some couplers on HPLC although other analytical tools indicate them to be >95% pure.<sup>d</sup>This information is not available.

TABLE II

| Coupler | Substituent Constant Values <sup>a,b</sup> |      |                |      |      |      |                |      |                |       |          |       |       |
|---------|--------------------------------------------|------|----------------|------|------|------|----------------|------|----------------|-------|----------|-------|-------|
|         | X <sub>1</sub>                             |      | X <sub>2</sub> |      | Y    |      | G <sub>1</sub> |      | G <sub>2</sub> |       | Σ Parent |       |       |
|         | σ                                          | π    |                | σ    | π    |      | σ              | π    |                | σ     | π        | σ     | π     |
| C-1     | 0.23                                       | 0.71 | 0.23           | 0.71 | 0.23 | 0.71 | 0.23           | 0.71 | 0.21           | 8.46  | 1.13     | 11.30 | 0.00  |
| C-2     | 0.23                                       | 0.71 | 0.23           | 0.71 | 0.23 | 0.71 | 0.23           | 0.71 | 0.21           | 7.81  | 1.13     | 10.65 | 1.55  |
| C-3     | 0.23                                       | 0.71 | 0.23           | 0.71 | 0.23 | 0.71 | 0.23           | 0.71 | 0.21           | 7.81  | 1.13     | 10.65 | 0.26  |
| C-4     | 0.23                                       | 0.71 | 0.23           | 0.71 | 0.23 | 0.71 | 0.23           | 0.71 | 0.21           | 6.08  | 1.13     | 8.92  | 9.06  |
| C-5     | 0.23                                       | 0.71 | 0.23           | 0.71 | 0.23 | 0.71 | 0.23           | 0.71 | 0.21           | 7.81  | 1.13     | 10.65 | 6.08  |
| C-6     | -0.17                                      | 0.56 | 0.23           | 0.71 | 0.23 | 0.71 | -0.17          | 0.56 | 0.21           | 6.08  | 0.33     | 8.62  | 0.26  |
| C-7     | 0.23                                       | 0.71 | 0.23           | 0.71 | 0.23 | 0.71 | 0.23           | 0.71 | 0.37           | 6.53  | 1.29     | 9.37  | 6.08  |
| C-8     | 0.23                                       | 0.71 | 0.23           | 0.71 | 0.23 | 0.71 | 0.23           | 0.71 | 0.57           | 4.60  | 1.49     | 7.44  | 0.26  |
| C-9     | 0.23                                       | 0.71 | 0.23           | 0.71 | 0.23 | 0.71 | 0.23           | 0.71 | 0.57           | 4.60  | 1.49     | 7.44  | 0.61  |
| C-10    | 0.23                                       | 0.71 | 0.23           | 0.71 | 0.23 | 0.71 | 0.23           | 0.71 | 0.57           | 4.60  | 1.49     | 7.44  | 5.37  |
| C-11    | 0.23                                       | 0.71 | 0.23           | 0.71 | 0.23 | 0.71 | 0.23           | 0.71 | 0.57           | 4.60  | 1.49     | 7.44  | 0.39  |
| C-12    | 0.23                                       | 0.71 | 0.23           | 0.71 | 0.23 | 0.71 | 0.23           | 0.71 | 0.57           | 4.60  | 1.49     | 7.44  | 6.21  |
| C-13    | 0.23                                       | 0.71 | 0.23           | 0.71 | 0.23 | 0.71 | 0.23           | 0.71 | 0.21           | 7.81  | 1.13     | 10.65 | 3.75  |
| C-14    | 0.23                                       | 0.71 | 0.23           | 0.71 | 0.23 | 0.71 | 0.23           | 0.71 | 0.21           | 6.43  | 1.59     | 10.69 | 1.39  |
| I-1     | 0.23                                       | 0.71 | 0.23           | 0.71 | 0.23 | 0.71 | 0.23           | 0.71 | 0.57           | -0.38 | 1.49     | 2.46  | 6.08  |
| I-2     | 0.23                                       | 0.71 | 0.23           | 0.71 | 0.23 | 0.71 | 0.23           | 0.71 | 0.57           | -0.38 | 1.49     | 2.46  | 8.12  |
| I-3     | 0.23                                       | 0.71 | 0.23           | 0.71 | 0.23 | 0.71 | 0.23           | 0.71 | 0.57           | -0.38 | 1.49     | 2.46  | 11.37 |
| I-4     | 0.23                                       | 0.71 | 0.23           | 0.71 | 0.23 | 0.71 | 0.23           | 0.71 | 0.57           | -0.38 | 1.49     | 2.46  | 9.28  |
| I-5     | 0.23                                       | 0.71 | 0.23           | 0.71 | 0.23 | 0.71 | 0.23           | 0.71 | 0.57           | 0.25  | 1.49     | 3.09  | 6.08  |
| I-6     | 0.23                                       | 0.71 | 0.23           | 0.71 | 0.23 | 0.71 | 0.23           | 0.71 | 0.57           | 2.35  | 1.49     | 5.19  | 6.08  |
| I-7     | 0.23                                       | 0.71 | 0.23           | 0.71 | 0.23 | 0.71 | 0.23           | 0.71 | 0.57           | 2.26  | 1.49     | 5.10  | 6.08  |
| I-8     | 0.23                                       | 0.71 | 0.23           | 0.71 | 0.23 | 0.71 | 0.23           | 0.71 | 0.57           | 2.48  | 1.49     | 5.32  | 6.08  |
| I-9     | 0.23                                       | 0.71 | 0.23           | 0.71 | 0.23 | 0.71 | 0.23           | 0.71 | 0.57           | 1.87  | 1.49     | 4.71  | 6.08  |
| I-10    | 0.23                                       | 0.71 | 0.23           | 0.71 | 0.23 | 0.71 | 0.23           | 0.71 | 0.57           | 2.37  | 1.49     | 5.21  | 6.08  |
| I-11    | 0.23                                       | 0.71 | 0.23           | 0.71 | 0.23 | 0.71 | 0.23           | 0.71 | 0.57           | 2.37  | 1.49     | 5.21  | 9.80  |
| I-12    | 0.23                                       | 0.71 | 0.23           | 0.71 | 0.23 | 0.71 | 0.23           | 0.71 | 0.57           | 2.11  | 1.49     | 4.95  | 6.08  |
| I-13    | 0.23                                       | 0.71 | 0.23           | 0.71 | 0.23 | 0.71 | 0.23           | 0.71 | 0.57           | 1.93  | 1.49     | 4.77  | 6.08  |
| I-14    | 0.23                                       | 0.71 | 0.23           | 0.71 | 0.23 | 0.71 | 0.23           | 0.71 | 0.57           | 4.49  | 1.49     | 7.33  | 6.08  |
| I-15    | 0.23                                       | 0.71 | 0.23           | 0.71 | 0.23 | 0.71 | 0.23           | 0.71 | 0.57           | 4.60  | 1.49     | 7.44  | 6.08  |
| I-16    | 0.23                                       | 0.71 | 0.23           | 0.71 | 0.23 | 0.71 | 0.23           | 0.71 | 0.57           | 4.60  | 1.49     | 7.44  | 5.37  |
| I-17    | 0.23                                       | 0.71 | 0.23           | 0.71 | 0.23 | 0.71 | 0.23           | 0.71 | 0.57           | 4.60  | 1.49     | 7.44  | 11.37 |
| I-18    | 0.23                                       | 0.71 | 0.23           | 0.71 | 0.23 | 0.71 | 0.23           | 0.71 | 0.57           | 4.60  | 1.49     | 7.44  | 5.25  |
| I-19    | 0.23                                       | 0.71 | 0.23           | 0.71 | 0.23 | 0.71 | 0.23           | 0.71 | 0.57           | 4.60  | 1.49     | 7.44  | 9.28  |
| I-20    | 0.23                                       | 0.71 | 0.23           | 0.71 | 0.23 | 0.71 | 0.23           | 0.71 | 0.57           | 4.60  | 1.49     | 7.44  | 9.80  |

TABLE II-continued

| Coupler | Substituent Constant Values <sup>a,b</sup> |      |                |      |      |      |                |      |                |      |          |       |                      |   |
|---------|--------------------------------------------|------|----------------|------|------|------|----------------|------|----------------|------|----------|-------|----------------------|---|
|         | X <sub>1</sub>                             |      | X <sub>2</sub> |      | Y    |      | G <sub>1</sub> |      | G <sub>2</sub> |      | Σ Parent |       | Σ Z + R <sub>1</sub> |   |
|         |                                            | σ    | π              |      | σ    | π    |                | σ    | π              |      | σ        | π     |                      | σ |
| I-21    | 0.23                                       | 0.71 | 0.23           | 0.71 | 0.23 | 0.71 | 0.23           | 0.71 | 0.57           | 4.60 | 1.49     | 7.44  | 4.81                 |   |
| I-22    | 0.23                                       | 0.71 | 0.23           | 0.71 | 0.23 | 0.71 | 0.23           | 0.71 | 0.57           | 4.60 | 1.49     | 7.44  | 9.06                 |   |
| I-23    | 0.23                                       | 0.71 | 0.23           | 0.71 | 0.23 | 0.71 | 0.23           | 0.71 | 0.45           | 6.53 | 1.37     | 9.37  | 6.08                 |   |
| I-24    | 0.23                                       | 0.71 | 0.23           | 0.71 | 0.23 | 0.71 | 0.23           | 0.71 | 0.36           | 4.54 | 1.35     | 7.38  | 6.08                 |   |
| I-25    | 0.23                                       | 0.71 | 0.23           | 0.71 | 0.23 | 0.71 | 0.23           | 0.71 | 0.69           | 5.82 | 1.61     | 8.66  | 6.08                 |   |
| I-26    | 0.23                                       | 0.71 | 0.23           | 0.71 | 0.23 | 0.71 | 0.23           | 0.71 | 0.60           | 1.42 | 1.52     | 4.26  | 6.08                 |   |
| I-27    | 0.23                                       | 0.71 | 0.23           | 0.71 | 0.23 | 0.71 | 0.23           | 0.71 | 0.60           | 7.24 | 1.52     | 10.08 | 6.08                 |   |
| I-28    | 0.23                                       | 0.71 | 0.23           | 0.71 | 0.23 | 0.71 | 0.23           | 0.71 | 0.78           | 4.18 | 1.64     | 7.02  | 6.08                 |   |
| I-29    | 0.23                                       | 0.71 | 0.23           | 0.71 | 0.23 | 0.71 | 0.23           | 0.71 | 0.57           | 4.60 | 1.49     | 7.44  | 3.75                 |   |
| I-30    | 0.23                                       | 0.71 | 0.23           | 0.71 | 0.23 | 0.71 | 0.23           | 0.71 | 0.78           | 4.18 | 1.64     | 7.02  | 3.75                 |   |
| I-31    | 0.23                                       | 0.71 | 0.23           | 0.71 | 0.23 | 0.71 | 0.23           | 0.71 | 0.78           | 4.18 | 1.64     | 7.02  | 7.84                 |   |
| I-32    | 0.23                                       | 0.71 | 0.23           | 0.71 | 0.23 | 0.71 | 0.23           | 0.71 | 0.78           | 4.18 | 1.64     | 7.02  | 2.61                 |   |
| I-33    | 0.23                                       | 0.71 | 0.23           | 0.71 | 0.23 | 0.71 | 0.23           | 0.71 | 0.78           | 4.18 | 1.64     | 7.02  | 3.69                 |   |
| I-34    | 0.23                                       | 0.71 | 0.23           | 0.71 | 0.23 | 0.71 | 0.23           | 0.71 | 0.78           | 4.18 | 1.64     | 7.02  | 10.10                |   |
| I-35    | 0.23                                       | 0.71 | 0.23           | 0.71 | 0.23 | 0.71 | 0.23           | 0.71 | 0.78           | 4.18 | 1.64     | 7.02  | 9.06                 |   |

<sup>a</sup>Values for sigma and pi were found in published chemical literature (see for example "The Chemist Companion", A. J. Gordon and R. A. Ford, John Wiley & Sons, New York, 1972; "Progress in Physical Organic Chemistry, Volume 13", R. W. Taft, Ed., John Wiley & Sons, New York; and C. Hansch and A. J. Leo, in "Substituent Constants for Correlation Analysis in Chemistry and Biology", Wiley, New York, 1979), or pi values were calculated using the Medchem program (for a recent discussion of this method see Albert J. Leo, in "Comprehensive Medicinal Chemistry", edited by C. Hansch, P. G. Sammes, and J. B. Taylor, Pergamon Press, New York, Volume 4, 1990). The values for sigma<sub>para</sub> were used to estimate the value for substituents ortho to the pyrazolone nucleus. Σ Parent is the sum of the values of the substituent constants X<sub>1</sub>, X<sub>2</sub>, Y, G<sub>1</sub>, and G<sub>2</sub>.

Typically, the coupler is incorporated in a silver halide emulsion and the emulsion coated on a support to form part of a photographic element. Alternatively, the coupler can be incorporated at a location adjacent to the silver halide emulsion where, during development, the coupler will be in reactive association with development products such as oxidized color developing agent. Thus, as used herein, the term "associated therewith" signifies that the coupler is in the silver halide emulsion layer or in an adjacent location where, during processing, the coupler is capable of reacting with silver halide development products.

The photographic elements can be single color elements or multicolor elements. Multicolor elements contain dye image-forming units sensitive to each of the three primary regions of the spectrum. Each unit can be comprised of a single emulsion layer or of multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented

A typical multicolor photographic element comprises a support bearing a cyan dye image-forming unit comprised of at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler, at least one of the couplers in the element being a coupler of this invention. The element can contain additional layers, such as filter layers, interlayers, overcoat layers, subbing layers, and the like.

In the following discussion of suitable materials for use in the emulsions and elements of this invention, reference will be made to Research Disclosure, December 1989, Item 308119, published by Kenneth Mason Publications, Ltd., Dudley Annex, 12a North Street, Emsworth, Hampshire P010 7DQ, ENGLAND, which will be identified hereafter by the term "Research Dis-

closure." The contents of the Research Disclosure, including the patents and publications referenced therein, are incorporated herein by reference, and the Sections hereafter referred to are Sections of the Research Disclosure.

The silver halide emulsions employed in the elements of this invention can be either negative-working or positive-working. Suitable emulsions and their preparation as well as methods of chemical and spectral sensitization are described in Sections I through IV. Color materials and development modifiers are described in Sections V and XXI. Vehicles are described in Section IX, and various additives such as brighteners, antifogging agents, stabilizers, light absorbing and scattering materials, hardeners, coating aids, plasticizers, lubricants and matting agents are described, for example, in Sections V, VI, VIII, X, XI, XII, and XVI. Manufacturing methods are described in Sections XIV and XV, other layers and supports in Sections XIII and XVII, processing methods and agents in Sections XIX and XX, and exposure alternatives in Section XVIII.

Preferred color developing agents are p-phenylene diamines. Especially preferred are:  
 4-amino N,N-diethylaniline hydrochloride,  
 4-amino-3-methyl-N,N-diethylaniline hydrochloride,  
 4-amino-3-methyl-N-ethyl-N-(β-(methanesulfonamido)ethyl)aniline sesquisulfate hydrate,  
 4-amino-3-methyl-N-ethyl-N-(β-hydroxyethyl)aniline sulfate,  
 4-amino-3-β-(methanesulfonamido)ethyl-N,N-diethylaniline hydrochloride and  
 4-amino-N-ethyl-N-(2-methoxyethyl)-m-toluidine di-p-toluene sulfonic acid.

With negative working silver halide a negative image can be formed. Optionally positive (or reversal) image can be formed.

The magenta coupler described herein may be used in combination with other classes of magenta image couplers such as 3-acylamino-5-pyrazolones and heterocyclic couplers (e.g. pyrazoloazoles) such as those described in EP 285,274; U.S. Pat. No. 4,540,654; EP 119,860, or with other 5-pyrazolone couplers containing different ballasts or coupling-off groups such as those described in U.S. Pat. Nos. 4,301,235; 4,853,319 and

4,351,897. The coupler may also be used in association with yellow or cyan colored couplers (e.g. to adjust levels of interlayer correction) and with masking couplers such as those described in EP 213,490; Japanese Published Application 58-172,647; U.S. Pat. NO. 2,983,608; German Application DE 2,706,117C; U.K. Patent 1,530,272; Japanese Application A-113935; U.S. Pat. No. 4,070,191 and German Application DE 2,643,965. The masking couplers may be shifted or blocked.

The coupler may also be used in association with materials that accelerate or otherwise modify the processing steps e.g. of bleaching or fixing to improve the quality of the image. Bleach accelerators described in EP 193,389; EP 301,477; U.S. Pat. Nos. 4,163,669; 4,865,956; and 4,923,784 are particularly useful. Also contemplated is use of the coupler in association with nucleating agents, development accelerators or their precursors (UK Patent 2,097,140; U.K. Patent 2,131,188); electron transfer agents (U.S. Pat. Nos. 4,859,578; 4,912,025); antifogging and anti color-mixing agents such as derivatives of hydroquinones, aminophenols, amines, gallic acid; catechol; ascorbic acid; hydrazides; sulfonamidophenols; and non color-forming couplers. Suitable hydroquinone color fog inhibitors include, but are not limited to compounds disclosed in EP 69,070; EP 98,241; EP 265,808; Japanese Published Patent Applications 61/233,744; 62/178,250; and 62/178,257. In addition, specifically contemplated are 1,4-benzenedipentanoic acid, 2,5-dihydroxy- $\Delta$ ,  $\Delta$ ,  $\Delta$ ',  $\Delta$ '-tetramethyl-, dihexyl ester; 1,4-Benzenedipentanoic acid, 2-hydroxy-5-methoxy- $\Delta$ ,  $\Delta$ ',  $\Delta$ '-tetramethyl-, dihexyl ester; and 2,5-dimethoxy- $\Delta$ ,  $\Delta$ ',  $\Delta$ ',  $\Delta$ '-tetramethyl-, dihexyl ester. In addition, it is contemplated that materials of this invention may be used with so called liquid ultraviolet absorbers such as described in U.S. Pat Nos. 4,992,358; 4,975,360; and 4,587,346.

Various kinds of discoloration inhibitors can be used with materials of this invention. Typical examples of organic discoloration inhibitors include hindered phenols represented by hydroquinones, 6-hydroxychromans, 5-hydroxycoumarans, spirochromans, p-alkoxyphenols and bisphenols, gallic acid derivatives, methylenedioxybenzenes, aminophenols, hindered amines, and ether or ester derivatives obtained by silylation, alkylation or acylation of phenolic hydroxy groups of the above compounds. Also, metal complex salts represented by (bis-salicylaldoximato)nickel complex and (bis-N,N-dialkylthiocarbamato)nickel complex can be employed as a discoloration inhibitor. Specific examples of the organic discoloration inhibitors are described below. For instance, those of hydroquinones are disclosed in U.S. Pat Nos. 2,360,290; 2,418,613; 2,700,453; 2,701,197; 2,710,801; 2,816,028; 2,728,659; 2,732,300; 2,735,765; 3,982,944 and 4,430,425; and British Patent 1,363,921; and so on; 6-hydroxychromans, 5-hydroxycoumarans, spirochromans are disclosed in U.S. Pat. Nos. 3,432,300; 3,573,050; 3,574,627; 3,698,909 and 3,764,337; and Japanese Published Patent Application 52-152,225; and so on; spiroindanes are disclosed in U.S. Pat. No. 4,360,589; those of p-alkoxyphenols are disclosed in U.S. Pat No. 2,735,765; British Patent 2,066,975; Japanese Published Patent Applications 59-010,539 and 57-019,765; and so on; hindered phenols are disclosed, for example, in U.S. Pat Nos. 3,700,455; 4,228,235; Japanese Published Patent Applications 52-072,224 and 52-006,623; and so on; gallic acid derivatives, methylenedioxybenzenes and aminophenols are

disclosed in U.S. Pat Nos. 3,457,079; 4,332,886; and Japanese Published Patent Application 56-021,144, respectively; hindered amines are disclosed U.S. Pat Nos. 3,336,335; 4,268,593; British Patents 1,326,889; 1,354,313 and 1,410,846; Japanese Published Patent Applications 51-001,420; 58-114,036; 59-053,846; 59-078,344; and so on; those of ether or ester derivatives of phenolic hydroxy groups are disclosed in U.S. Pat Nos. 4,155,765; 4,174,220; 4,254,216; 4,279,990; Japanese Published Patent Applications 54-145,530; 55006,321; 58-105,147; 59-010,539; 57-037,856; 53-003,263 and so on; and those of metal complexes are disclosed in U.S. Pat. Nos. 4,050,938 and 4,241,155.

For example, the coupler of the invention may be used to replace all or part of the image coupler or may be added to one or more of the other layers in a color negative photographic element comprising a support bearing the following layers from top to bottom:

(1) one or more overcoat layers containing ultraviolet absorber(s);

(2) a two-coat yellow pack with a fast yellow layer containing "Coupler 1": Benzoic acid, 4-chloro-3((2-(4-ethoxy-2,5-dioxo-3-(phenylmethyl)-1-imidazolidinyl)-3-(4-methoxyphenyl)-1,3-dioxopropyl) amino)-, dodecyl ester and a slow yellow layer containing the same compound together with "Coupler 2": Propanoic acid, 2-[[5-[[4-[2-[[2,4-bis(1,1-dimethylpropyl)phenoxyl]acetyl]amino]-5-[(2,2,3,3,4,4,4-heptafluoro-1-oxobutyl) amino]-4-hydroxyphenoxy]-2,3-dihydroxy-6-[(propylamino) carbonyl]phenyl]thio]-1,3,4-thiadiazol-2-yl]thio], methyl ester and "Coupler 3": 1-((dodecyloxy) carbonyl) ethyl (3-chloro-4-(3-(2-chloro-4-((1-tridecanoylethoxy) carbonyl) anilino)-3-oxo-2-((4)(5)(6)-(phenoxy carbonyl)-1H-benzotriazol-1-yl)propanoyl)amino)benzoate;

(3) an interlayer containing fine metallic silver;

(4) a triple-coat magenta pack with a fast magenta layer containing "Coupler 4": Benzamide, 3-((2-(2,4-bis(1,1-dimethylpropyl)phenoxy)-1-oxobutyl)amino)-N-(4,5-dihydro-5-oxo-1-(2,4,6-trichlorophenyl)-1H-pyrazol-3-yl)-, "Coupler 5": Benzamide, 3-((2-(2,4-bis(1,1-dimethylpropyl)phenoxy)-1-oxobutyl)amino)-N-(4',5'-dihydro-5'-oxo-1'-(2,4,6-trichlorophenyl) (1,4-bi-1H-pyrazol)-3'-yl)-, "Coupler 6": Carbamic acid, (6-((3-(dodecyloxy)propyl) amino)carbonyl)-5-hydroxy-1-naphthalenyl)-2-methylpropyl ester, "Coupler 7": Acetic acid, ((2-((3-((3-(dodecyloxy)propyl)amino)carbonyl)-4-hydroxy-8-(((2-methylpropoxy)carbonyl)amino)-1-naphthalenyl)oxy)ethyl)thio)-, and "Coupler 8": Benzamide, 3-((2-(2,4-bis(1,1-dimethylpropyl)phenoxy)-1-oxobutyl)amino)-N-(4,5-dihydro-4-((4-methoxyphenyl)azo)-5-oxo-1-(2,4,6-trichlorophenyl)-1H-pyrazol-3-yl)-, a mid-magenta layer and a slow magenta layer each containing "Coupler 9": a ternary copolymer containing by weight in the ratio 1:1:2 2-Propenoic acid butyl ester, styrene, and N-[1-(2,4,6-trichlorophenyl)-4,5-dihydro-5-oxo-1H-pyrazol-3-yl]-2-methyl-2-propenamide; and "Coupler 10": Tetradecanamide, N-(4-chloro-3-((4-((2,2-dimethyl-1-oxopropyl)amino)phenyl)azo)-4,5-dihydro-5-oxo-1(2,4,6-trichlorophenyl)-1H-pyrazol-3-yl)amino)phenyl)-, in addition to Couplers 3 and 8;

(5) an interlayer;

(6) a triple-coat cyan pack with a fast cyan layer containing Couplers 6 and 7; a mid-cyan containing Coupler 6 and "Coupler 11": 2,7-Naphthalenedisulfonic acid, 5-(acetylamino)-3-((4-(2-((3-(2,4-bis(1,1-dimethylpropyl)phenoxy)amino)carbonyl)-4-

hydroxy-1-naphthalenyl)oxyethoxy)phenyl)azo)-4-hydroxy-, disodium salt; and a slow cyan layer containing Couplers 2 and 6;

- (7) an undercoat layer containing Coupler 8; and
- (8) an antihalation layer.

In a color paper format, the coupler of the invention may suitably be used to replace all or a part of the image coupler or added to a layer in a photographic element such as one comprising a support bearing the following from top to bottom:

- (1) one or more overcoats;
- (2) a cyan layer containing "Coupler 1": Butanamide, 2-(2,4-bis(1,1-dimethylpropyl)phenoxy)-N-(3,5-dichloro-2-hydroxy-4-methylphenyl)-, "Coupler 2": Acetamide, 2-(2,4-bis(1,1-dimethylpropyl)phenoxy)-N-(b 3,5-dichloro-2-hydroxy-4-, and UV Stabilizers: Phenol, 2-(5-chloro-2H-benzotriazol-2-yl)-4,6-bis(1,1-dimethylpropyl)-; Phenol, 2-(2H-benzotriazol-2-yl)-4-(1,1-dimethylpropyl)-; Phenol, 2-(2H-benzotriazol-2-yl)-4-(1,1-dimethylpropyl)-6-(1-methylpropyl)-; and Phenol, 2-(2H-benzotriazol-2-yl)-4,6-bis(1,1-dimethylpropyl)- and a poly(t-butylacrylamide) dye stabilizer;
- (3) an interlayer;
- (4) a magenta layer containing "Coupler 3": Octanamide, 2-[2,4-bis(1,1-dimethylpropyl)phenoxy]-N-[2-(7-chloro-6-methyl-1H-pyrazolo[1,5-b][1,2,4]triazol-2-yl)propyl]- together with 1,1'-Spirobi(1H-indene), 2,2',3,3'-tetrahydro-3,3',3'-tetramethyl-5,5',6,6'-tetrapropoxy-;
- (5) an interlayer; and

(6) a yellow layer containing "Coupler 4": 1-Imidazolidineacetamide, N-(5-((2-(2,4-bis(1,1-dimethylpropyl)phenoxy)-1-oxobutyl)amino)-2-chlorophenyl)-.alpha.-(2,2-dimethyl-1-oxopropyl)-4-ethoxy-2,5-dioxo-3-(phenylmethyl)-.

In a reversal medium, the coupler of the invention could be used to replace all or part of the image coupler or added to a layer in a photographic element such as one comprising a support and bearing the following layers from top to bottom:

- (1) one or more overcoat layers;
- (2) a nonsensitized silver halide containing layer;
- (3) a triple-coat yellow layer pack with a fast yellow layer containing "Coupler 1": Benzoic acid, 4-(1-((2-chloro-5-(dodecylsulfonyl)amino)phenyl)amino)carbonyl)-3,3-dimethyl-2-oxobutoxy-, 1-methylethyl ester; a mid yellow layer containing Coupler 1 and "Coupler 2": Benzoic acid, 4-chloro-3-[[2-[4-ethoxy-2,5-dioxo-3-(phenylmethyl)-1-imidazolidinyl]-4,4-dimethyl-1,3-dioxopentyl]amino]-, dodecylester; and a slow yellow layer also containing Coupler 2;

- (4) an interlayer;
- (5) a layer of fine-grained silver;
- (6) an interlayer;

(7) a triple-coated magenta pack with a fast magenta layer containing "Coupler 3": 2-Propenoic acid, butyl ester, polymer with N-[1-(2,5-dichlorophenyl)-4,5-dihydro-5-oxo-1H-pyrazol-3-yl]-2-methyl-2-propenamide; "Coupler 4": Benzamide, 3-((2-(2,4-bis(1,1-dimethylpropyl)phenoxy)-1-oxobutyl)amino)-N-(4,5-dihydro-5-oxo-1-(2,4,6-trichlorophenyl)-1H-pyrazol-3-yl)-; and "Coupler 5": Benzamide, 3-((2,4-bis(1,1-dimethylpropyl)phenoxy)acetyl)amino)-N-(4,5-dihydro-5-oxo-1-(2,4,6-trichlorophenyl)-1H-pyrazol-3-yl)-; and containing the stabilizer 1,1'-Spirobi(1H-indene), 2,2',3,3'-tetrahydro-3,3',3'-tetramethyl-5,5',6,6'-tetrapropoxy-; and in the slow magenta layer Couplers 4 and 5 with the same stabilizer;

(8) one or more interlayers possibly including fine-grained nonsensitized silver halide;

(9) a triple-coated cyan pack with a fast cyan layer containing "Coupler 6": Tetradecanamide, 2-(2-cyano-phenoxy)-N-(4-((2,2,3,3,4,4,4-heptafluoro-1-oxobutyl)amino)-3-hydroxyphenyl)-; a mid cyan containing "Coupler 7": Butanamide, N-(4-((2-(2,4-bis(1,1-dimethylpropyl)phenoxy)-1-oxobutyl)amino)-2-hydroxy-phenyl)-2,2,3,3,4,4,4-heptafluoro- and "Coupler 8":

- 10 Hexanamide, 2-(2,4-bis(1,1-dimethylpropyl)phenoxy)-N-(4-((2,2,3,3,4,4,4-heptafluoro-1-oxobutyl)amino)-3-hydroxyphenyl)-;
- 15 (10) one or more interlayers possibly including fine-grained nonsensitized silver halide; and
- (11) an antihalation layer.

The couplers of the invention are useful with gelatin hardeners known to the art, such as 1,2-bis (vinylsulfonyl-acetamido)ethane, 2,4-dichloro-6-hydroxy-s-triazine, triacryloyltriazine, and pyridinium, 1-(4-morpholinylcarbonyl)-4-(2-sulfoethyl)-hydroxide, inner salt. Further, it is contemplated that the couplers of the invention would be particularly useful with so-called rapid acting hardeners, such as described in U.S. Pat. No. 4,877,724 and allowed application U.S. Ser. No. 07/770,393.

The couplers may also be used in combination with filter dye layers comprising colloidal silver sol or yellow and/or magenta filter dyes, either as oil-in-water dispersions, latex dispersions or as solid particle disper-

30 sions. Additionally, they may be used with "smearing" couplers (e.g. as described in U.S. Pat. No. 4,366,237; EP 96,570; U.S. Pats. No. 4,420,556; and 4,543,323). Also, the couplers may be blocked or coated in protected form as described, for example, in Japanese Application 61/258,249 or U.S. Pat. No. 5,019,492.

The coupler may further be used in combination with image-modifying compounds such as "Developer Inhibitor-Releasing" compounds (DIR's). DIR's useful in conjunction with the couplers of the invention are

- 40 known in the art and examples are described in U.S. Pat. Nos. 3,137,578; 3,148,022; 3,148,062; 3,227,554; 3,384,657; 3,379,529; 3,615,506; 3,617,291; 3,620,746; 3,701,783; 3,733,201; 4,049,455; 4,095,984; 4,126,459; 4,149,886; 4,150,228; 4,211,562; 4,248,962; 4,259,437; 4,362,878; 4,409,323; 4,477,563; 4,782,012; 4,962,018; 4,500,634; 4,579,816; 4,607,004; 4,618,571; 4,678,739; 4,746,600; 4,746,601; 4,791,049; 4,857,447; 4,865,959; 4,880,342; 4,886,736; 4,937,179; 4,946,767; 4,948,716; 4,952,485; 4,956,269; 4,959,299; 4,966,835; 4,985,336 as well as in patent publications GB 1,560,240; GB 2,007,662; GB 2,032,914; GB 2,099,167; DE 2,842,063, DE 2,937,127; DE 3,636,824; DE 3,644,416 as well as the following European Patent Publications: 272,573; 335,319; 336,411; 346,899; 362,870; 365,252; 365,346; 373,382; 376,212; 377,463; 378,236; 384,670; 396,486; 401,612; 401,613.

Such compounds are also disclosed in "Developer-Inhibitor-Releasing (DIR) Couplers for Color Photography," C. R. Barr, J. R. Thirtle and P. W. Vittum in 60 *Photographic Science and Engineering*, Vol. 13, p. 174 (1969), incorporated herein by reference. Generally, the developer inhibitor-releasing (DIR) couplers include a coupler moiety and an inhibitor coupling-off moiety (IN). The inhibitor-releasing couplers may be of the time-delayed type (DIAR couplers) which also include a timing moiety or chemical switch which produces a delayed release of inhibitor. Examples of typical inhibitor moieties are: oxazoles, thiazoles, diazoles, triazoles,

oxadiazoles, thiadiazoles, oxathiazoles, thiatriazoles, benzotriazoles, tetrazoles, benzimidazoles, indazoles, isoindazoles, mercaptotetrazoles, selenotetrazoles, mercaptobenzothiazoles, selenobenzothiazoles, mercaptobenzoxazoles, selenobenzoxazoles, mercaptobenzimidazoles, selenobenzimidazoles, benzodiazoles, mercaptooxazoles, mercaptothiadiazoles, mercaptothiazoles, mercaptotriazoles, mercaptooxadiazoles, mercaptodiazoles, mercaptooxathiazoles, telleurotetrazoles or benzisodiazoles. In a preferred embodiment, the inhibitor moiety or group is selected from the following formulas:



wherein  $R_I$  is selected from the group consisting of straight and branched alkyls of from 1 to about 8 carbon atoms, benzyl and phenyl groups and said groups containing at least one alkoxy substituent;  $R_{II}$  is selected from  $R_I$  and  $-SR_I$ ;  $R_{III}$  is a straight or branched alkyl group of from 1 to about 5 carbon atoms and  $m$  is from 1 to 3; and  $R_{IV}$  is selected from the group consisting of hydrogen, halogens and alkoxy, phenyl and carbonamido groups,  $-COOR_V$  and  $-NHOOR_V$  wherein  $R_V$  is selected from substituted and unsubstituted alkyl and aryl groups.

Although it is typical that the coupler moiety included in the developer inhibitor-releasing coupler forms an image dye corresponding to the layer in which

it is located, it may also form a different color as one associated with a different film layer. It may also be useful that the coupler moiety included in the developer inhibitor-releasing coupler forms colorless products and/or products that wash out of the photographic material during processing (so-called "universal" couplers).

As mentioned, the developer inhibitor-releasing coupler may include a timing group which produces the time-delayed release of the inhibitor group such as groups utilizing the cleavage reaction of a hemiacetal (U.S. Pat. No. 4,146,396, Japanese Applications 60-249148; 60-249149); groups using an intramolecular nucleophilic substitution reaction (U.S. Pat. No. 4,248,962); groups utilizing an electron transfer reaction along a conjugated system (U.S. Pat. Nos. 4,409,323; 4,421,845; Japanese Applications 57-188035; 58-98728; 58-209736; 58-209738) groups utilizing ester hydrolysis (German Patent Application (OLS) No. 2,626,315); groups utilizing the cleavage of imino ketals (U.S. Pat. No. 4,546,073); groups that function as a coupler or reducing agent after the coupler reaction (U.S. Pat. Nos. 4,438,193; 4,618,571) and groups that combine the features described above. It is typical that the timing group or moiety is of one of the formulas:



wherein IN is the inhibitor moiety, Z is selected from the group consisting of nitro, cyano, alkylsulfonyl; sulfamoyl ( $-SO_2NR_2$ ); and sulfonamido ( $-NRSO_2R$ ) groups;  $n$  is 0 or 1; and  $R_{VI}$  is selected from the group consisting of substituted and unsubstituted alkyl and phenyl groups. The oxygen atom of each timing group is bonded to the coupling-off position of the respective coupler moiety of the DIAR.

Suitable developer inhibitor-releasing couplers for use in the present invention include, but are not limited to, the following:



5,447,830

43

44

-continued

D2



D3



D4



D5



D6





-continued

D7



D8

It is also contemplated that the concepts of the present invention may be employed to obtain reflection color prints as described in *Research Disclosure*, Nov. 1979, Item 18716, available from Kenneth Mason Publications, Ltd, Dudley Annex, 12a North Street, Emsworth, Hampshire P0101 7DQ, England, incorporated herein by reference. Materials of the invention may be coated on pH adjusted support as described in U.S. Pat. No. 4,917,994; with epoxy solvents (EP 0 164 961); with nickel complex stabilizers (U.S. Pat. Nos. 4,346,165; 4,540,653 and 4,906,559 for example); with ballasted chelating agents such as those in U.S. Pat. No. 4,994,359 to reduce sensitivity to polyvalent cations such as calcium; and with stain reducing compounds such as described in U.S. Pat. No. 5,068,171. Other compounds useful in combination with the invention are disclosed in Japanese Published Applications 90-072,629, 40 90-072,630; 90-072,631; 90-072,632; 90-072,633; 90-072,634; 90-077,822; 90-078,229; 90-078,230; 90-079,336; 90-079,337; 90-079,338; 90-079,690; 90-079,691; 90-080,487; 90-080,488; 90-080,489; 90-080,490; 90-080,491; 90-080,492; 90-080,494; 90-085,928; 90-086,669; 90-086,670; 90-087,360; 90-087,361; 90-087,362; 90-087,363; 90-087,364; 90-088,097; 90-093,662; 90-093,663; 90-093,664; 90-093,665; 90-093,666; 90-093,668; 90-094,055; 90-094,056; 90-103,409; 83-62,586; 83-09,959.

If desired, the photographic element can be used in conjunction with an applied magnetic layer as described in *Research Disclosure*, Nov. 1992, Item 34390 published by Kenneth Mason Publications, Ltd., Dudley Annex, 12a North Street, Emsworth, Hampshire P010 7DQ,

45 ENGLAND. Thus, materials of the invention may be employed in conjunction with a photographic material where a relatively transparent film containing magnetic particles is incorporated into the material. The materials of this invention function well in such a combination and give excellent photographic results. Examples of such magnetic films are well known and are described for example in U.S. Patent 4,990,276 and EP 459,349 which are incorporated herein by reference.

50 As disclosed in these publications, the particles can be of any type available such as ferro- and ferri-magnetic oxides, complex oxides with other metals, ferrites etc. and can assume known particulate shapes and sizes, may contain dopants, and may exhibit the pH values known in the art. The particles may be shell coated and may be applied over the range of typical laydown.

55 The embodiment is not limited with respect to binders, hardeners, antistatic agents, dispersing agents, plasticizers, lubricants and other known additives.

60 The couplers of the invention are especially suited for use in combination with these magnetic layers. The layer may suitably be located on the side of the photographic material substrate opposite to the silver halide emulsions and may be employed to magnetically record any desired information. One notable deficiency attributed to such a layer is that the particle layer tends to absorb blue light when light is shined through the processed negative to create a reflective color print. This distorts the color otherwise obtainable without the layer unless needed corrections are made. This also reduces the light transmission during printing so that

the printing time must be increased for comparable results. In one embodiment of the invention, the coupler of the present invention may be incorporated in the magenta dye forming layer to replace all or part of the conventional coupler since the invention coupler contains less unwanted blue absorption and can therefore help counteract the undesirable impact of the magnetic layer. Also, if a yellow colored magenta mask is employed, the amount of the mask may be diminished. On the other hand, if all or a portion of the blue absorption can be tolerated, considering the reduction achieved by the invention, then additional amounts of photographically useful groups which generate dye with blue absorbance, such as development inhibitors, can be added to improve sharpness, color and other important photographic properties.

Especially useful in this invention are tabular grain silver halide emulsions. Specifically contemplated tabular grain emulsions are those in which greater than 50 percent of the total projected area of the emulsion grains are accounted for in the case of silver bromide or silver bromoiodide by tabular grains having a thickness of less than 0.3 micron (0.5 micron for blue sensitive emulsion) and an average tabularity (T) of greater than 25 (preferably greater than 100), where the term "tabularity" is employed in its art recognized usage as

$$T = ECD/t^2$$

where

ECD is the average equivalent circular diameter of the tabular grains in micrometers and

t is the average thickness in micrometers of the tabular grains.

The average useful ECD of photographic emulsions can range up to about 10 micrometers, although in practice emulsion ECD's seldom exceed about 4 micrometers. Since both photographic speed and granularity increase with increasing ECD's, it is generally preferred to employ the smallest tabular grain ECD's compatible with achieving aim speed requirements.

Emulsion tabularity increases markedly with reductions in tabular grain thickness. It is generally preferred that aim tabular grain projected areas be satisfied by thin ( $t < 0.2$  micrometers) tabular grains. To achieve the lowest levels of granularity it is preferred that aim tabular grain projected areas be satisfied with ultrathin ( $t < 0.06$  micrometers) tabular grains. Tabular grain thicknesses typically range down to about 0.02 micrometers. However, still lower tabular grain thicknesses are contemplated. For example, Daubendiek et al U.S. Pat. No. 4,672,027 reports a 3 mole percent iodide tabular grain silver bromoiodide emulsion having a grain thickness of 0.017 micrometers. Ultrathin tabular grain high chloride emulsions are disclosed by Maskasky U.S. Ser. No. 763,030 filed Sep. 20, 1991, now allowed.

As noted above tabular grains of less than the specified thickness account for at least 50 percent of the total grain projected area of the emulsion. To maximize the advantages of high tabularity it is generally preferred that tabular grains satisfying the stated thickness criterion account for the highest conveniently attainable percentage of the total grain projected area of the emulsion. For example, in preferred emulsions, tabular grains satisfying the stated thickness criteria above account for at least 70 percent of the total grain projected area. In the highest performance tabular grain emulsions, tabu-

lar grains satisfying the thickness criteria above account for at least 90 percent of total grain projected area.

Suitable tabular grain emulsions can be selected from among a variety of conventional teachings, such as those of the following: Research Disclosure, Item 22534, Jan. 1983, published by Kenneth Mason Publications, Ltd., Emsworth, Hampshire P010 7DD, England; U.S. Pat. Nos. 4,439,520; 4,414,310; 4,433,048; 4,643,966; 4,647,528; 4,665,012; 4,672,027; 4,678,745; 4,693,964; 4,713,320; 4,722,886; 4,755,456; 4,775,617; 4,797,354; 4,801,522; 4,806,461; 4,835,095; 4,853,322; 4,914,014; 4,962,015; 4,985,350; 5,061,069,5,061,616, 5,210,013 and PCT Ser. No. 93/06521, published Apr. 1, 1993.

15 The following examples are included for a further understanding of this invention.

#### Coating Method 1 (4-Equivalent Couplers)

Photographic elements were prepared by coating a 20 gel-subbed, polyethylene-coated paper support with a photosensitive layer containing a silver chloride emulsion at 0.2865 g Ag/m<sup>2</sup> for the 4-equivalent coupler (C-1). Gelatin was coated at 1.238 g/m<sup>2</sup> and C-1 was coated at 0.549 mmol/m<sup>2</sup>. Comparison coupler C-1 was 25 dispersed with the following addenda (weight percent of coupler): dibutyl phthalate (50%), Addendum-1 (42.6%), Addendum-2 (10%). The photosensitive layer was overcoated with a protective layer containing gelatin at 1.08 g/m<sup>2</sup> and bisvinylsulfonylmethyl ether hardener at 2 weight percent based on total gelatin.

#### Coating Method 2 (2-Equivalent Couplers)

Photographic elements were prepared by coating a 35 gel-subbed, polyethylene-coated paper support with a photosensitive layer containing a silver chloride emulsion at 0.172 g Ag/m<sup>2</sup>, gelatin at 1.238 g/m<sup>2</sup>, and a magenta image coupler indicated below at 0.38 mmol/m<sup>2</sup> dispersed in the following addenda (weight percent of coupler): tricresyl phosphate (108%), Addendum-2 (10%), Addendum-3 (115%) and ethyl acetate layer containing gelatin at 1.08 g/m<sup>2</sup> and bisvinylsulfonylmethyl ether hardener at 2 weight percent based on total gelatin. The levels of coupler and silver were chosen to approximate the sensitometry of the 45 4-equivalent check coupler.

#### Coating Method 3 (4-Equivalent Couplers)

Photographic elements were prepared by coating a 50 gel-subbed, polyethylene-coated paper support with a photosensitive layer containing a silver chloride emulsion at 0.2854 g Ag/m<sup>2</sup> for the 4-equivalent coupler C-1. Gelatin was coated at 1.615 g/m<sup>2</sup> and C-1 was coated at 0.560 mmol/m<sup>2</sup>. Comparison coupler C-1 was dispersed with the following addenda (weight percent of coupler): dibutyl phthalate (50%), Addendum-1 (42.6%), and Addendum-2 (10%). The photosensitive layer was overcoated with an ultraviolet absorbing layer containing gelatin at 1.335 g/m<sup>2</sup>, Addendum-5 at 0.732 g/m<sup>2</sup>, Addendum-6 at 0.129 g/m<sup>2</sup>, and Addendum-2 at 0.059 g/m<sup>2</sup>, and with a protective layer containing gelatin at 1,399 g/m<sup>2</sup> and bisvinyl sulfonyl methyl ether hardener at 2 weight percent based on total gelatin.

#### Coating Method 4 (2-Equivalent Couplers)

Photographic elements were prepared by coating a 65 gel-subbed, polyethylene-coated, neutral pH-adjusted, paper support as described in U.S. Pat No. 4,917,994 with a photosensitive layer containing a silver chloride

emulsion at 0.172 g Ag/m<sup>2</sup>, gelatin at 1.614 g/m<sup>2</sup>, and the magenta image coupler was coated at 0.329 mmol/m<sup>2</sup> dispersed in the following addenda (weight percent of coupler): tricresyl phosphate (100%), Addendum-3 (117%), and Addendum-4 (16.7%) and ethyl acetate (300%). The photosensitive layer was over-coated with an ultraviolet absorbing layer containing gelatin at 1.335 g/m<sup>2</sup>, Addendum-5 at 0.732 g/m<sup>2</sup>, Addendum-6 at 0.129 g/m<sup>2</sup>, and Addendum-2 at 0.059

g/m<sup>2</sup>, and with a protective layer containing gelatin at 1.399 g/m<sup>2</sup> and bisvinyl sulfonyl methyl ether hardener at 2 weight percent based on total gelatin.

## Coating Method 5

The photographic elements were prepared by coating the following layers in the order listed on a resin-coated neutral pH-adjusted, paper support as described in U.S. Pat No. 4,917,994:

|           |                                |                          |
|-----------|--------------------------------|--------------------------|
| 1st Layer | Gelatin                        | 3.23 g/m <sup>2</sup>    |
| 2nd Layer | Gelatin                        | 1.61 g/m <sup>2</sup>    |
|           | Coupler Disperison             | 0.32 mmol/m <sup>2</sup> |
|           | Silver Chloride Emulsion       | 0.172 g/m <sup>2</sup>   |
| 3rd Layer | Gelatin                        | 1.33 g/m <sup>2</sup>    |
|           | Addendum-5                     | 0.73 g/m <sup>2</sup>    |
|           | Addendum-6                     | 0.13 g/m <sup>2</sup>    |
| 4th Layer | Gelatin                        | 1.40 g/m <sup>2</sup>    |
|           | Bis(vinylsulfonylmethyl) ether | 0.14 g/m <sup>2</sup>    |

---

**Addendum-I:**



## Addendum-2:



### Addendum-3:



## Addendum-4



## Addendum-5



## Addendum-6



-continued

Addendum-7



Addendum-8



Addendum-9



Addendum-10



Addendum-11



Addendum-12

-continued

Addendum-13



Addendum-14



Addendum-15



Addendum-16



Addendum-17

-continued



## Processing Method 1

Samples of each element were imagewise exposed for 1/10 of a second through a graduated-density test object, then processed in color developer at 35° C. (45 seconds in a color developer, 45 seconds in the bleach-fix bath) washed and dried.

| Color Developer (pH 10.04)                                                           |         |
|--------------------------------------------------------------------------------------|---------|
| Triethanolamine                                                                      | 12.41 g |
| Lithium sulfate                                                                      | 2.70 g  |
| N, N-Diethylhydroxylamine (85% solution)                                             | 5.40 g  |
| 1-Hydroxyethylidene-1,1-di-phosphonic acid (60%)                                     | 1.16 g  |
| 4-Amino-3-methyl-N-ethyl-N-( $\beta$ -methanesulfonamido)ethylanilinesulfate hydrate | 5.00 g  |
| Potassium carbonate (anhydrous)                                                      | 21.16 g |
| Potassium bicarbonate                                                                | 2.79 g  |
| Potassium chloride                                                                   | 1.60 g  |
| Potassium bromide                                                                    | 7.0 mg  |
| Stilbene whitening agent                                                             | 2.30 g  |
| Surfactant                                                                           | 1 mL    |
| Water to make                                                                        | 1.0 L   |
| Bleach-Fix Bath (pH 6.8)                                                             |         |
| Ammonium thiosulfate                                                                 | 104 g   |
| Sodium hydrogen sulfite                                                              | 13 g    |
| Ferric ammonium ethylenediamine tetraacetic acid (EDTA)                              | 65.5 g  |
| EDTA                                                                                 | 6.56 g  |
| Ammonium hydroxide (28%)                                                             | 27.9 mL |
| Water to make                                                                        | 1 L     |

## Processing Method 2

The photographic elements were given stepwise exposures and processed as follows at 35° C.:

|                      |            |
|----------------------|------------|
| Developer            | 45 seconds |
| Bleach-Fix           | 45 seconds |
| Wash (running water) | 90 seconds |

The developer and bleach-fix were of the following compositions:

| Developer                                                                        |           |
|----------------------------------------------------------------------------------|-----------|
| Water                                                                            | 700.00 mL |
| Triethanolamine                                                                  | 12.41 g   |
| Blankophor REU™ (Mobay Corp.)                                                    | 2.30 g    |
| Lithium polystyrene sulfonate (30%)                                              | 0.30 g    |
| N,N-Diethylhydroxylamine (85%)                                                   | 5.40 g    |
| Lithium sulfate                                                                  | 2.70 g    |
| N-[2-[(4-amino-3-methylphenyl)ethylamino]ethyl]methanesulfonamide, sesquisulfate | 5.00 g    |
| 1-Hydroxyethyl-1,1-diphosphonic acid (60%)                                       | 0.81 g    |
| Potassium carbonate, anhydrous                                                   | 21.16 g   |

-continued

|    |                                                                 |           |
|----|-----------------------------------------------------------------|-----------|
| 20 | Potassium chloride                                              | 1.60 g    |
|    | Potassium bromide                                               | 7.00 mg   |
|    | Water to make                                                   | 1.00 L    |
|    | pH @ 26.7° C. adjusted to 10.4 ± 0.05                           |           |
|    | <u>Bleach-Fix</u>                                               |           |
| 25 | Water                                                           | 700.00 mL |
|    | Solution of ammonium thiosulfate (56.4%) +                      | 127.40 g  |
|    | Ammoniumsulfite (4%)                                            |           |
|    | Sodium metabisulfite                                            | 10.00 g   |
|    | Acetic acid (glacial)                                           | 10.20 g   |
|    | Solution of ammonium ferric ethylenediaminetetraacetate (44%) + | 110.40 g  |
|    | ethylenediaminetetraacetic acid (3.5%)                          |           |
|    | Water to make                                                   | 1.00 L    |
| 30 | pH @ 26.7° C. adjusted to 6.7                                   |           |

## EXAMPLE 1

35 Hue  
 The couplers were coated by Methods 1 (4-equivalent) and 2 (2-equivalent) and processed by Method 1. The spectral characteristics ( $\lambda_{max}$ ) for the 4-amino-3-methyl-N-ethyl-N- $\beta$ -(methanesulfonamido)ethylaniline dyes of the representative couplers are summarized in Table III. It is clearly evident that the dye hues of invention couplers are bathochromic to the comparison couplers C-2 through C-7 dye hue, which is desirable for better color reproduction. Check couplers C-8 through C-12 also have acceptable hue, but the thermal stability of the couplers in unprocessed coatings is inferior to couplers of the invention (see raw stock keeping).

50 Raw Stock Keeping (RSK)  
 The couplers were coated as described above. The coatings were incubated in a 49° C./50% relative humidity oven for 2 weeks. The coatings were processed as described. The differences in minimum density, relative to check coatings kept at -15° C., are reported in Table III. As is seen, the unprocessed couplers of the invention are uniformly more stable than the comparison 2-equivalent check couplers, especially when comparing the invention couplers to the check couplers with improved hue (couplers C-8 to C-12).

55 60 In order to evaluate the combined effect of a coupler on hue and raw stock keeping (RSK), a composite score for each coupler tested was determined based on the following:

| 65 | Hue     | Score | RSK    |
|----|---------|-------|--------|
|    | ≥544    | 5     | <.20   |
|    | 539-543 | 3     | .2-.39 |

-continued

| Hue     | Score | RSK        |
|---------|-------|------------|
| 534-538 | 1     | .4-.59     |
| <534    | 0     | $\geq .60$ |

The composite scoring shows that the invention couplers exhibit a distinct improvement over the comparison couplers which would not have been expected. Check coupler C-1 has a good composite score but this coupler is a four-equivalent coupler having the prior art recognized problem of low coupling efficiency compared to the 2 equivalent couplers tested.

TABLE III

| Coupler | Type      | Hue and Raw Stock Data                |                                                |                    |
|---------|-----------|---------------------------------------|------------------------------------------------|--------------------|
|         |           | Hue<br>( $\lambda_{\text{max}}$ , nm) | RSK<br>( $\Delta D_{\text{min}}$ )<br>Two Week | Composite<br>Score |
| C-1     | Check     | 539                                   | 0.16                                           | 8                  |
| C-2     | Check     | 536                                   | na                                             | —                  |
| C-3     | Check     | 536                                   | 0.88                                           | 1                  |
| C-4     | Check     | 536                                   | na                                             | —                  |
| C-5     | Check     | 537                                   | 1.04                                           | 1                  |
| C-6     | Check     | 530                                   | na                                             | —                  |
| C-7     | Check     | 536                                   | 0.25                                           | 4                  |
| C-8     | Check     | 543                                   | 0.43                                           | 4                  |
| C-9     | Check     | 544                                   | 0.60                                           | 5                  |
| C-10    | Check     | 544                                   | 0.62                                           | 5                  |
| C-11    | Check     | 543                                   | 0.53                                           | 4                  |
| C-12    | Check     | 543                                   | 0.50                                           | 4                  |
| I-1     | Invention | 543                                   | 0.32                                           | 6                  |
| I-2     | Invention | 542                                   | 0.36                                           | 6                  |
| I-5     | Invention | 543                                   | 0.34                                           | —                  |
| I-6     | Invention | 543                                   | 0.29                                           | —                  |
| I-7     | Invention | 543                                   | 0.36                                           | 6                  |
| I-8     | Invention | 543                                   | 0.33                                           | 6                  |
| I-9     | Invention | 543                                   | 0.33                                           | 6                  |
| I-10    | Invention | 543                                   | 0.29                                           | 6                  |
| I-11    | Invention | 542                                   | 0.29                                           | 6                  |
| I-12    | Invention | 543                                   | 0.36                                           | 6                  |
| I-13    | Invention | 543                                   | 0.24                                           | 6                  |
| I-14    | Invention | 543                                   | 0.36                                           | 6                  |
| I-15    | Invention | 543                                   | 0.31                                           | 6                  |
| I-16    | Invention | 544                                   | 0.26                                           | 6                  |
| I-17    | Invention | 542                                   | 0.32                                           | 6                  |
| I-18    | Invention | 543                                   | 0.28                                           | 6                  |
| I-19    | Invention | 542                                   | 0.36                                           | 6                  |
| I-20    | Invention | 542                                   | na                                             | —                  |
| I-21    | Invention | 544                                   | na                                             | —                  |
| I-22    | Invention | 543                                   | 0.36                                           | 6                  |
| I-23    | Invention | 540                                   | 0.19                                           | 8                  |
| I-24    | Invention | 540                                   | na                                             | —                  |
| I-25    | Invention | 541                                   | 0.24                                           | 6                  |
| I-26    | Invention | 540                                   | 0.17                                           | 8                  |
| I-27    | Invention | 539                                   | 0.39                                           | 6                  |
| I-28    | Invention | 543                                   | 0.12                                           | 8                  |

## EXAMPLE 2

## Reduction of Calcium Ion Sensitivity

The coupling kinetics of a number of coupler dispersions with oxidized color developer (4-Amino-3-methyl-N-ethyl-N-( $\beta$ -methanesulfonamido)ethylanilinesesquisulfate hydrate) are determined as a function of the calcium ion concentration by competition with the hydroxide deamination of the oxidized color developer. These competition kinetics are run in a buffer solution (0.0125M of 4-carboxybenzenesulfonamide) containing a maximum of 0.36M potassium ion and a series of calcium ion concentrations (from 0 to 0.16M) with varying potassium ion to maintain a constant total cation level. Known, limited amounts of color developer and excess oxidant (potassium ferricyanide) are added to the dilute dispersions in the buffered media. The relative dye yields are determined spectrophotometrically as a function of the coupler concentration. After corrections for interfering densities, the coupling rate constants are calculated from previously determined rates for oxidized developer deamination as a function of pH by use of standard competition kinetics analysis. For each coupler dispersion the log of the coupling rate constant is plotted as a function of the log of the calcium ion concentration. For all of these coupler dispersions there is a region wherein the coupling rate constants are independent of calcium ion concentration ( $k_1$ ) and a region of decreasing coupling rate with increasing calcium ion concentration. The point of intersection of the calcium ion dependent region and the calcium ion independent region is defined as the threshold, and is reported as the log of the calcium ion concentration for that point. The relative threshold normalizes the values with respect to check coupler C-14. Couplers with a relative threshold of less than 1.00 are more sensitive to calcium ion than couplers with a relative threshold of greater than 1.00. The threshold, the absolute rate constants with no added calcium ion ( $k_1$ ), at a calcium ion concentration of 0.1M ( $k_2$ ), and the difference ( $\Delta \log k$ ) are presented in Table IV below. From this information is calculated a relative sensitivity toward calcium ion by normalizing the  $\Delta \log k$  information with respect to check coupler C-14. Couplers with a relative sensitivity of greater than 1.00 are more sensitive toward calcium ion than couplers with a relative threshold of less than 1.00.

As is clearly seen, couplers represented by the invention are less sensitive to the presence of calcium ion in the process than the check couplers. For instance, in comparison to check coupler C-3, invention coupler I-28 has a threshold value nearly 1000 times larger, and is 12 times less sensitive toward calcium ion at a concentration of 0.1M.

TABLE IV

| Coupler | Type      | Calcium Ion Sensitivity. |                    |            |            |                 |                      |
|---------|-----------|--------------------------|--------------------|------------|------------|-----------------|----------------------|
|         |           | Threshold                | Relative Threshold | $\log k_1$ | $\log k_2$ | $\Delta \log k$ | Relative Sensitivity |
| C-2     | Check     | -4.30                    | 0.13               | 2.34       | 1.22       | -1.12           | 1.15                 |
| C-3     | Check     | -5.29                    | 0.01               | 2.90       | 1.33       | -1.57           | 3.24                 |
| C-5     | Check     | -4.80                    | 0.04               | 2.35       | 1.25       | -1.10           | 1.09                 |
| C-13    | Check     | -4.55                    | 0.07               | 2.98       | 1.35       | -1.63           | 3.72                 |
| C-14    | Check     | -3.40                    | 1.00               | 2.60       | 1.54       | -1.06           | 1.00                 |
| I-15    | Invention | -2.48                    | 8.32               | 3.16       | 2.59       | -0.57           | 0.32                 |
| I-23    | Invention | -2.75                    | 4.47               | 2.99       | 2.32       | -0.67           | 0.41                 |
| I-25    | Invention | -2.63                    | 5.88               | 3.36       | 2.84       | -0.52           | 0.29                 |
| I-28    | Invention | -2.30                    | 12.59              | 3.02       | 2.54       | -0.48           | 0.26                 |
| I-29    | Invention | -3.11                    | 1.95               | 3.13       | 2.32       | -0.81           | 0.56                 |

TABLE IV-continued

| Coupler | Type      | Threshold | Relative  |            |            | Relative<br>Sensitivity |      |
|---------|-----------|-----------|-----------|------------|------------|-------------------------|------|
|         |           |           | Threshold | $\log k_1$ | $\log k_2$ |                         |      |
| I-30    | Invention | -3.20     | 1.59      | 3.14       | 2.31       | -0.83                   | 0.59 |

## EXAMPLE 3

Thermal Stability of the Dyes (Fade from an Initial Density of 1.0)

The couplers were coated by Methods 1 (4-equivalent) and 2 (2-equivalent) and processed by Method 1, and the data obtained after treatment under the specified conditions is listed in Table V. The invention couplers give a magenta dye which is much less prone to fade under dry oven conditions than state of the art coupler C-1. The small gains in green density for the invention couplers may be due to an increased covering power phenomenon.

Thermal Stability of the Couplers (Yellowing of the Areas of Minimum Density)

The couplers were coated and processed as described above, and the data obtained after treatment under the specified conditions is listed in Table V. It is clearly evident that couplers of invention are much less prone to discoloration than the check couplers.

TABLE V

| Thermal Stability of the Magenta Dyes and Couplers <sup>a,b</sup> |           |                              |                              |                                   |                                   |
|-------------------------------------------------------------------|-----------|------------------------------|------------------------------|-----------------------------------|-----------------------------------|
| Coupler                                                           | Type      | Dry Oven                     | Wet Oven                     | Dry Oven                          | Wet Oven                          |
|                                                                   |           | Fade<br>( $\Delta$ from 1.0) | Fade<br>( $\Delta$ from 1.0) | Yellowing<br>( $\Delta$ from 0.0) | Yellowing<br>( $\Delta$ from 0.0) |
| C-1                                                               | Check     | -0.22                        | -0.12                        | 0.11                              | 0.15                              |
| C-3                                                               | Check     | -0.07                        | -0.01                        | 0.13                              | 0.04                              |
| I-15                                                              | Invention | -0.03                        | 0.02                         | 0.09                              | 0.03                              |
| I-23                                                              | Invention | 0.00                         | 0.01                         | 0.08                              | 0.03                              |
| I-25                                                              | Invention | -0.03                        | 0.03                         | 0.09                              | 0.03                              |
| I-26                                                              | Invention | -0.02                        | 0.01                         | 0.09                              | 0.03                              |
| I-28                                                              | Invention | 0.00                         | 0.02                         | 0.08                              | 0.02                              |

<sup>a</sup>Dry Oven Conditions: 4 weeks, 77° C./15% relative humidity.

<sup>b</sup>Wet Oven Conditions: 4 weeks, 60° C./70% relative humidity.

## EXAMPLE 4

## Coupler Activity:

The couplers were coated by Methods 1 (4-equivalent) and 2 (2-equivalent) and processed as described by Method 1. The data obtained after treatment under the specified conditions is listed in Table VI. The speed and contrast of the invention couplers were greater than check couplers C-3 and C-5.

## Leuco-Dye Formation:

The couplers were coated and processed as described above. The processed coatings were exposed to heat and the results are tabulated below. The large increases in density for the check coupler are indicative of the decomposition of a stable leuco-dye to give additional magenta dye upon heat treatment. The couplers of the invention do not form a stable leuco-dyes under these rapid access conditions. Therefore, couplers of the invention do not require Lippman fine grain silver halide for rapid machine processing, a distinct advantage over comparison coupler C-1.

10  
15

TABLE VI

| Coupler | Type      | Coupler Activity and Unwanted Formation of Stable Leuco-Dyes <sup>a,b</sup> |          |                                     |                                     |
|---------|-----------|-----------------------------------------------------------------------------|----------|-------------------------------------|-------------------------------------|
|         |           | Speed<br>at<br>$\Delta = 1.0$                                               | Contrast | Dry Oven<br>( $\Delta$ from<br>1.7) | Wet Oven<br>( $\Delta$ from<br>1.7) |
| C-2     | Check     | na                                                                          | na       | 0.23                                | 0.26                                |
| C-3     | Check     | 138                                                                         | 2.38     | -0.01                               | 0.00                                |
| C-5     | Check     | 136                                                                         | 2.58     | 0.04                                | 0.07                                |
| I-15    | Invention | 145                                                                         | 2.76     | 0.01                                | 0.07                                |
| I-23    | Invention | 141                                                                         | 2.74     | 0.02                                | 0.04                                |
| I-25    | Invention | 146                                                                         | 2.80     | 0.03                                | 0.02                                |
| I-26    | Invention | 143                                                                         | 2.74     | 0.04                                | 0.03                                |
| I-28    | Invention | 144                                                                         | 2.74     | 0.05                                | 0.04                                |

<sup>a</sup>Dry Oven Conditions: 1 week, 77° C./15% relative humidity.

<sup>b</sup>Wet Oven Conditions: 1 week, 60° C./70% relative humidity.

## EXAMPLE 5

Comparison coupler C-1 was coated as described in Coating Method 3 while two-equivalent samples were prepared as described in Coating Method 4. The couplers were processed by Method 2 and were subjected

25

45 to routine testing for the following characteristics:

## Contrast

Contrast is defined as the slope of a line on a plot of density vs. log exposure connecting the points at which the log exposure is 0.3 less and 0.3 greater, respectively, than the log exposure that gave a density of 1.0. The dye hue is defined as the wavelength in nanometers of maximum absorption. Half bandwidth (HBW) is the width of the absorption spectrum in nanometers at half peak height.

## Light Stability

Dye light stability is the change in density to green light from an initial density of 1.0 after exposure to simulated daylight at an intensity of 50 klux for a period of four weeks.

## Dark Stability

Dye dark stability is the change in density to green light from an initial density of 1.0 after incubation in the dark at 75° C. and 50% relative humidity for a period of four weeks. Yellowing is the change in blue density in a minimum density area after the same incubation conditions.

60  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
2510  
2511  
2512  
2513  
2514  
2515  
2516  
2517  
2518  
2519  
2520  
2521  
2522  
2523  
2524  
2525  
2526  
2527  
2528  
2529  
2530  
2531  
2532  
2533  
2534  
2535  
2536  
2537  
2538  
2539  
2540  
2541  
2542  
2543  
2544  
2545  
2546  
2547  
2548  
2549  
2550  
2551  
2552  
2553  
2554  
2555  
2556  
2557  
2558  
2559  
2560  
2561  
2562  
2563  
2564  
2565  
2566  
2567  
2568  
2569  
2570  
2571  
2572  
2573  
2574  
2575  
2576  
2577  
2578  
2579  
2580  
2581  
2582  
2583  
2584  
2585  
2586  
2587  
2588  
2589  
2590  
2591  
2592  
2593  
2594  
2595  
2596  
2597  
2598  
2599  
25100  
25101  
25102  
25103  
25104  
25105  
25106  
25107  
25108  
25109  
25110  
25111  
25112  
25113  
25114  
25115  
25116  
25117  
25118  
25119  
25120  
25121  
25122  
25123  
25124  
25125  
25126  
25127  
25128  
25129  
25130  
25131  
25132  
25133  
25134  
25135  
25136  
25137  
25138  
25139  
25140  
25141  
25142  
25143  
25144  
25145  
25146  
25147  
25148  
25149  
25150  
25151  
25152  
25153  
25154  
25155  
25156  
25157  
25158  
25159  
25160  
25161  
25162  
25163  
25164  
25165  
25166  
25167  
25168  
25169  
25170  
25171  
25172  
25173  
25174  
25175  
25176  
25177  
25178  
25179  
25180  
25181  
25182  
25183  
25184  
25185  
25186  
25187  
25188  
25189  
25190  
25191  
25192  
25193  
25194  
25195  
25196  
25197  
25198  
25199  
25200  
25201  
25202  
25203  
25204  
25205  
25206  
25207  
25208  
25209  
25210  
25211  
25212  
25213  
25214  
25215  
25216  
25217  
25218  
25219  
25220  
25221  
25222  
25223  
25224  
25225  
25226  
25227  
25228  
25229  
25230  
25231  
25232  
25233  
25234  
25235  
25236  
25237  
25238  
25239  
25240  
25241  
25242  
25243  
25244  
25245  
25246  
25247  
25248  
25249  
25250  
25251  
25252  
25253  
25254  
25255  
25256  
25257  
25258  
25259  
25260  
25261  
25262  
25263  
25264  
25265  
25266  
25267  
25268  
25269  
25270  
25271  
25272  
25273  
25274  
25275  
25276  
25277  
25278  
25279  
25280  
25281  
25282  
25283  
25284  
25285  
25286  
25287  
25288  
25289  
25290  
25291  
25292  
25293  
25294  
25295  
25296  
25297  
25298  
25299  
25300  
25301  
25302  
25303  
25304  
25305  
25306  
25307  
25308  
25309  
25310  
25311  
25312  
25313  
25314  
25315  
25316  
25317  
25318  
25319  
25320  
25321  
25322  
25323  
25324  
25325  
25326  
25327  
25328  
25329  
25330  
25331  
25332  
25333  
25334  
25335  
25336  
25337  
25338  
25339  
25340  
25341  
25342  
25343  
25344  
25345  
25346  
25347  
25348  
25349  
25350  
25351  
25352  
25353  
25354  
25355  
25356  
25357  
25358  
25359  
25360  
25361  
25362  
25363  
25364  
25365  
25366  
25367  
25368  
25369  
25370  
25371  
25372  
25373  
25374  
25375  
25376  
25377  
25378  
25379  
25380  
25381  
25382  
25383  
25384  
25385  
25386  
25387  
25388  
25389  
25390  
25391  
25392  
25393  
25394  
25395  
25396  
25397  
25398  
25399  
25400  
25401  
25402  
25403  
25404  
25405  
25406  
25407  
25408  
25409  
25410  
25411  
25412  
25413  
25414  
25415  
25416  
25417  
25418  
25419  
25420  
25421  
25422  
25423  
25424  
25425  
25426  
25427  
25428  
25429  
25430  
25431  
25432  
25433  
25434  
25435  
25436  
25437  
25438  
25439  
25440  
25441  
25442  
25443  
25444  
25445  
25446  
25447  
25448  
25449  
25450  
25451  
25452  
25453  
25454  
25455  
25456  
25457  
25458  
25459  
25460  
25461  
25462  
25463  
25464  
25465  
25466  
25467  
25468  
25469  
25470  
25471  
25472  
25473  
25474  
25475  
25476  
25477  
25478  
25479  
25480  
25481  
25482  
25483  
25484  
25485  
25486  
25487  
25488  
25489  
25490  
25491  
25492  
25493  
25494  
25495  
25496  
25497  
25498  
25499  
25500  
25501  
25502  
25503  
25504  
25505  
25506  
25507  
25508  
25509  
25510  
25511  
25512  
25513  
25514  
25515  
25516  
25517  
25518  
25519  
25520  
25521  
25522  
25523  
25524  
25525  
25526  
25527  
25528  
25529  
25530  
25531  
25532  
25533  
25534  
25535  
25536  
25537  
25538  
25539  
25540  
25541  
25542  
25543  
25544  
25545  
25546  
25547  
25548  
25549  
25550  
25551  
25552  
25553  
25554  
25555  
25556  
25557  
25558  
25559  
25560  
25561  
25562  
25563  
25564  
25565  
25566  
25567  
25568  
25569  
25570  
25571  
25572  
25573  
25574  
25575  
25576  
25577  
25578  
25579  
25580  
25581  
25582  
25583  
25584  
25585  
25586  
25587  
25588  
25589  
25590  
25591  
25592  
25593  
25594  
25595  
25596  
25597  
25598  
25599  
25600  
25601  
25602  
25603  
25604  
25605  
25606  
25607  
25608  
25609  
25610  
25611  
25612  
25613  
25614  
25615  
25616  
25617  
25618  
25619  
25620  
25621  
25622  
25623  
25624  
25625  
25626  
25627  
25628  
25629  
25630  
25631  
25632  
25633  
25634  
25635  
25636  
25637  
25638  
25639  
25640  
25641  
25642  
25643  
25644  
25645  
25646  
25647  
25648  
25649  
25650  
25651  
25652  
25653  
25654  
25655  
25656  
25657  
25658  
25659  
25660  
25661  
25662  
25663  
25664  
25665  
25666  
25667  
25668  
25669  
25670  
25671  
25672  
25673  
25674  
25675  
25676  
25677  
25678  
25679  
25680  
25681  
25682  
25683  
25684  
25685  
25686  
25687  
25688  
25689  
25690  
25691  
25692  
25693  
25694  
25695  
25696  
25697  
25698  
25699  
25700  
25701  
25702  
25703  
25704  
25705  
25706  
25707  
25708  
25709  
25710  
25711  
25712  
25713  
25714  
25715  
25716  
25717  
25718  
25719  
25720  
25721  
25722  
25723  
25724  
25725  
25726  
25727  
25728  
25729  
25730  
25731  
25732  
25733  
25734  
25735  
25736  
25737  
25738  
25739  
25740  
25741  
25742  
25743  
25744  
25745  
25746  
25747  
25748  
25749  
25750  
25751  
25752  
25753  
25754  
25755  
25756  
25757  
25758  
25759  
25760  
25761  
25762  
25763  
25764  
25765  
25766  
25767  
25768  
25769  
25770  
25771  
25772  
25773  
25774  
25775  
25776  
25777  
25778  
25779  
25780  
25781  
25782  
25783  
25784  
25785  
25786  
25787  
25788  
25789  
25790  
25791  
25792  
25793  
25794  
25795  
25796  
25797  
25798  
25799  
25800  
25801  
25802  
25803  
25804  
25805  
25806  
25807  
25808  
25809  
25810  
25811  
25812  
25813  
25814  
25815  
25816  
25817  
25818  
25819  
25820  
25821  
25822  
25823  
25824  
25825  
25826  
25827  
25828  
25829  
25830  
25831  
25832  
25833  
25834  
25835  
25836  
25837  
25838  
25839  
25840  
25841  
25842  
25843  
25844  
25845  
25846  
25847  
25848  
25849  
25850  
25851  
25852  
25853  
25854  
25855  
25856  
25857  
25858  
25859  
25860  
25861  
25862  
25863  
25864  
25865  
25866  
25867  
25868  
25869  
25870  
25871  
25872  
25873  
25874  
25875  
25876  
25877  
25878  
25879  
25880  
25881  
25882  
25883  
25884  
25885  
25886  
25887  
25888  
25889  
25890  
25891  
25892  
25893  
25894  
25895  
25896  
25897  
25898  
25899  
25900  
25901  
2

TABLE VII

| Coupler | Type      | Hue and Raw Stock Data            |                                          |                    |
|---------|-----------|-----------------------------------|------------------------------------------|--------------------|
|         |           | Hue<br>(λ <sub>max</sub> ,<br>nm) | RSK<br>(Δ D <sub>min</sub> )<br>Two Week | Composite<br>Score |
| C-1     | Check     | 539                               | 0.09                                     | 8                  |
| C-2     | Check     | 536                               | 0.53                                     | 2                  |
| C-5     | Check     | 537                               | 0.44                                     | 2                  |
| I-28    | Invention | 543                               | 0.12                                     | 8                  |
| I-31    | Invention | 542                               | 0.25                                     | 6                  |
| I-32    | Invention | 542                               | 0.25                                     | 6                  |
| I-33    | Invention | 542                               | 0.26                                     | 6                  |
| I-34    | Invention | 542                               | 0.29                                     | 6                  |
| I-35    | Invention | 542                               | 0.15                                     | 8                  |

The composite scoring shows that the invention couplers exhibit a distinct improvement over the comparison couplers which would not have been expected. Check coupler C-1 has a good composite score but this coupler is a four-equivalent coupler having the prior art recognized problem of low coupling efficiency compared to the 2 equivalent couplers tested.

TABLE VIII

| Coupler | Type   | Coupler Evaluation Data |                     |                    |
|---------|--------|-------------------------|---------------------|--------------------|
|         |        | Contrast                | Dye Light Stability | Dye Dark Stability |
| C-1     | Check  | 2.64                    | -0.73               | -0.13              |
| C-2     | Check  | 1.45                    | -0.91               | 0.18               |
| C-5     | Check  | 2.56                    | -0.52               | 0.01               |
| I-28    | Inven. | 2.76                    | -0.64               | 0.02               |
| I-31    | Inven. | 2.69                    | -0.56               | 0.01               |
| I-32    | Inven. | 2.64                    | -0.68               | 0.00               |
| I-33    | Inven. | 2.61                    | -0.65               | 0.00               |
| I-34    | Inven. | 2.76                    | -0.61               | -0.01              |
| I-35    | Inven. | 2.73                    | -0.59               | 0.00               |

A comparison of the results of Table VIII shows that the invention provides couplers with improved activity (as measured by the contrast), dye stability, and yellowing performance relative to the check couplers. Although check coupler C-5 provides comparable dye stability and yellowing performance, its hue is undesirable as was shown in Table VII. As was shown previously in Example 4, Table VI, check coupler C-2 is prone to leuco-dye formation as evidenced both by its poor contrast and dye density gain upon dark keeping.

#### EXAMPLE 6

The example described the use of the invention couplers with {100} silver chloride tabular emulsion as prepared as described in EP 534,395. The emulsions were then coated by Method 5 on a resin coated paper support and processed by Method 2.

#### Preparation of Photographic Elements

Each of the coupler dispersions used consisted of a disperse phase of the composition shown in Table IX and a dispersion medium comprising aqueous gelatin and an emulsifying agent. The dispersions were emulsified by methods well known in the photographic art.

TABLE IX

| Disperse Phase Composition |                                                                       |
|----------------------------|-----------------------------------------------------------------------|
| A                          | I-31, 30%; Addendum-3, 35%; Addendum-4, 5%; tricresyl phosphate, 30%  |
| B                          | I-31, 30%; Addendum-7, 40%; tricresyl phosphate, 30%                  |
| C                          | I-31, 30%; Addendum-1, 40%; tricresyl phosphate, 30%                  |
| D                          | I-31, 30%; Addendum-3, 40%; tricresyl phosphate, 30%                  |
| E                          | I-31, 30%; Addendum-7, 20%; Addendum-8, 20%; tricresyl phosphate, 30% |

TABLE IX-continued

| Disperse Phase Composition |                                                                              |
|----------------------------|------------------------------------------------------------------------------|
| F                          | I-31, 30%; Addendum-7, 20%; Addendum-3, 20%; tricresyl phosphate, 30%        |
| G                          | I-31, 30%; Addendum-7, 30%; Addendum-9, 10%; tricresyl phosphate, 30%        |
| H                          | I-31, 30%; Addendum-7, 35%; Addendum-4, 5%; tricresyl phosphate, 30%         |
| I                          | I-31, 30%; Addendum-3, 35%; Addendum-4, 5%; tris(2-ethylhexyl)phosphate, 30% |

#### Photographic Tests on Coating Examples 601 to 609

The material was processed as described above and the following photographic characteristics were determined: D-max (the maximum density to light of the color complimentary to the dye color); D-min (the minimum density); and Speed (the relative log exposure required to yield a density of 1.0). These values for each example are tabulated in Table X.

TABLE X

|    | Example No. | Dispersion | D-max | D-min | Speed |
|----|-------------|------------|-------|-------|-------|
| 25 | 601         | A          | 2.13  | 0.21  | 240   |
|    | 602         | B          | 2.46  | 0.30  | 252   |
|    | 603         | C          | 1.36  | 0.29  | 214   |
|    | 604         | D          | 2.44  | 0.30  | 250   |
|    | 605         | E          | 2.45  | 0.32  | 254   |
| 30 | 606         | F          | 2.45  | 0.27  | 255   |
|    | 607         | G          | 2.48  | 0.29  | 255   |
|    | 608         | H          | 2.24  | 0.24  | 242   |
|    | 609         | I          | 2.15  | 0.21  | 241   |

Table X demonstrates that the invention couplers are useful in combination with {100} silver chloride tabular emulsions in a variety of dispersion formulations commonly used for color paper reflection print materials.

#### EXAMPLE 7

This example shows the usefulness of the invention couplers in a variety of dispersion formulations. The emulsions were then coated by Method 5 on a resin coated paper support and processed by Method 2.

#### Preparation of Photographic Elements

Each of the coupler dispersions used consisted of a disperse phase of the composition shown in Table XI and a dispersion medium comprising aqueous gelatin and an emulsifying agent. The dispersions were emulsified by methods well known in the photographic art.

TABLE XI

| Disperse Phase Composition |                                                                                                                                               |
|----------------------------|-----------------------------------------------------------------------------------------------------------------------------------------------|
| J                          | I-31, 30%; Addendum-3, 17.5%; Addendum-7, 8.75%; Addendum-10, 8.75%; Addendum-4, 5%; tricresyl phosphate, 30%                                 |
| K                          | I-31, 30%; Addendum-3, 17.5%; Addendum-7, 17.5%; Addendum-4, 5%; tris(2-ethylhexyl)phosphate, 30%                                             |
| L                          | I-31, 30%; Addendum-3, 17.5%; Addendum-11, 17.5%; Addendum-4, 5%; tris(2-ethylhexyl)phosphate, 30%                                            |
| M                          | I-31, 30%; Addendum-3, 17.5%; Addendum-10, 17.5%; Addendum-4, 5%; tris(2-ethylhexyl)phosphate, 30%                                            |
| N                          | I-31, 30%; Addendum-3, 17.5%; Addendum-12, 17.5%; Addendum-4, 5%; tris(2-ethylhexyl)phosphate, 30%                                            |
| O                          | I-31, 30%; Addendum-3, 17.5%; Addendum-13, 17.5%; Addendum-4, 5%; tris(2-ethylhexyl)phosphate, 30%                                            |
| P                          | I-31, 30%; Addendum-3, 17.5%; Addendum-14, 17.5%; Addendum-4, 5%; tris(2-ethylhexyl)phosphate, 30%                                            |
| Q                          | I-31, 30%; Addendum-3, 17.5%; Addendum-1, 17.5%; Addendum-4, 5%; tris(2-ethylhexyl)phosphate, 30%                                             |
| R                          | I-31, 30%; Addendum-3, 17.5%; 1,2-benzenedicarboxylic acid, bis(2-ethoxyethyl) ester, 17.5%; Addendum-4, 5%; tris(2-ethylhexyl)phosphate, 30% |

TABLE XI-continued

| Disperse Phase Composition |                                                                                                                                                         |    |  |  |  |
|----------------------------|---------------------------------------------------------------------------------------------------------------------------------------------------------|----|--|--|--|
| S                          | I-31, 30%; Addendum-3, 17.5%; 1,2-benzenedicarboxylic acid, bis(2-(2-ethoxyethoxy)ethyl) ester, 17.5%; Addendum-4, 5%; tris(2-ethylhexyl)phosphate, 30% | 5  |  |  |  |
| T                          | I-31, 30%; Addendum-3, 25%; Addendum-15, 10%; Addendum-4, 5%; tris(2-ethylhexyl)phosphate, 30%                                                          |    |  |  |  |
| U                          | I-31, 30%; Addendum-3, 25%; Addendum-16, 10%; Addendum-4, 5%; tris(2-ethylhexyl)phosphate, 30%                                                          | 10 |  |  |  |
| V                          | I-31, 30%; Addendum-3, 35%; Addendum-4, 5%; tris(2-ethylhexyl)phosphate, 30%                                                                            |    |  |  |  |
| W                          | I-31, 30%; Addendum-3, 35%; Addendum-4, 5%; dibutyl phthalate, 30%                                                                                      | 15 |  |  |  |
| X                          | I-31, 30%; Addendum-3, 35%; Addendum-4, 5%; 1,2-benzenedicarboxylic acid, bis(1,1-diethylpropyl) ester, 30%                                             |    |  |  |  |
| Y                          | I-31, 30%; Addendum-3, 35%; Addendum-4, 5%; Addendum-17, 30%                                                                                            | 20 |  |  |  |

## Photographic Tests on Coating Examples 701 to 716

The material was processed as described above and the following photographic characteristics were determined: D-max (the maximum density to light of the color complimentary to the dye color); D-min (the minimum density); and Speed (the relative log exposure required to yield a density of 1.0). These values for each example are tabulated in Table XII.

TABLE XII

| Example No. | Dispersion | D-max | D-min | Speed | 35 |
|-------------|------------|-------|-------|-------|----|
| 701         | J          | 2.55  | 0.09  | 144   |    |
| 702         | K          | 2.46  | 0.09  | 145   |    |
| 703         | L          | 2.48  | 0.09  | 145   |    |
| 704         | M          | 2.48  | 0.09  | 145   |    |
| 705         | N          | 2.48  | 0.09  | 146   |    |
| 706         | O          | 2.49  | 0.09  | 146   | 40 |
| 707         | P          | 2.50  | 0.09  | 145   |    |
| 708         | Q          | 2.39  | 0.09  | 137   |    |
| 709         | R          | 2.49  | 0.10  | 146   |    |
| 710         | S          | 2.50  | 0.09  | 145   | 45 |
| 711         | T          | 2.43  | 0.09  | 139   |    |
| 712         | U          | 2.42  | 0.09  | 140   |    |
| 713         | V          | 2.46  | 0.10  | 141   |    |
| 714         | W          | 2.57  | 0.10  | 140   |    |
| 715         | X          | 2.40  | 0.10  | 133   | 50 |
| 716         | Y          | 2.43  | 0.10  | 133   |    |

Table XII demonstrates that the invention couplers are useful in a variety of dispersion formulations commonly used for color paper reflection print materials.

The invention has been described in detail with particular reference to preferred embodiments thereof, but it will be understood that variations and modifications can be effected within the spirit and scope of the invention.

What is claimed is:

1. A photographic element comprising a support bearing at least one silver halide emulsion layer having associated therewith a 5-pyrazolone photographic coupler represented by the formula:



wherein

- substituents X<sub>1</sub>, X<sub>2</sub>, Y, G<sub>1</sub>, and G<sub>2</sub> are individually selected from the group consisting of halogen, alkyl, alkoxy, aryloxy, acylamino, alkylthio, arylthio, sulfonamido, sulfamoyl, sulfamido, carbamoyl, diacylamino, alkoxy carbonyl, aryloxycarbonyl, alkoxy sulfonyl, aryloxysulfonyl, alkylsulfonyl, alkylsulfoxyl, arylsulfoxyl, arylsulfonyl, arylsulfonyl, alkoxycarbonylamino, aryloxycarbonylamino, alkylureido, arylureido, acyloxy, nitro, cyano, trifluoromethyl and carboxy and, in the case of X<sub>1</sub>, X<sub>2</sub> and Y, hydrogen;
- a, b, and c are individually integers from 0 to 3 provided that "a" cannot be an integer which, combined with the selection of X<sub>1</sub> and X<sub>2</sub>, allows the number of chloride substituents on the ring containing G<sub>1</sub> to exceed 3;
- R<sub>1</sub> is selected from the group consisting of G<sub>1</sub> and hydroxyl;
- Z is an amine group of the formula:



wherein R<sub>2</sub> is selected from the group consisting of hydrogen, alkyl, alkenyl, aryl, acyl, and heterocyclic; A is carbon and d is 1;

B is comprised of

- an atom of oxygen, nitrogen, sulfur, or carbon bonded to A, said atom also bonded to
- a substituent selected from the group consisting of alkyl, aryl, and heterocyclic groups,

wherein, when said atom bonded to A is carbon, B has the formula:



wherein R<sub>3</sub>, R<sub>4</sub>, and R<sub>5</sub> are individually selected from the group consisting of hydrogen, halogen, alkyl, aryl, heterocyclic group and W, wherein W is selected from the group consisting of -OR<sub>6</sub>, -SR<sub>6</sub>, and -NR<sub>7</sub>R<sub>8</sub>, wherein R<sub>6</sub> is selected from the group consisting of alkyl, aryl, and heterocyclic groups, and R<sub>7</sub> and R<sub>8</sub> are individually selected from the group consisting of hydrogen, alkyl, aryl, acyl, alkylsulfonyl, arylsulfonyl and heterocyclic group, provided that, when A is carbon, at least one of R<sub>3</sub>, R<sub>4</sub>, and R<sub>5</sub> is not hydrogen or alkyl and

provided that two of R<sub>3</sub>, R<sub>4</sub>, and R<sub>5</sub> may join to form an aliphatic, aromatic, or heterocyclic ring and that in the case of an aromatic ring the remaining member of R<sub>3</sub>, R<sub>4</sub>, and R<sub>5</sub> is an aromatic pi bond, and in the case of a nonaromatic unsaturated aliphatic or heterocyclic ring the remaining member may be a bond forming part of a double bond in the ring; and

- e) the sum of the sigma values for X<sub>1</sub>, X<sub>2</sub>, G<sub>1</sub>, G<sub>2</sub>, and Y is at least 1.3.
2. The element of claim 1 wherein B is bonded to A by an oxygen atom in B.
3. The element of claim 1 wherein B is bonded to A by a sulfur atom in B.
4. The element of claim 1 wherein B is bonded to A by a nitrogen atom in B.
5. The element of claim 1 wherein B is bonded to A by a carbon atom in B.
6. The element of claim 5 wherein at least one of R<sub>3</sub>, R<sub>4</sub> and R<sub>5</sub> is an aryloxy substituent.
7. The element of claim 6 wherein said aryloxy substituent is an alkylaryloxy substituent.
8. The element of claim 6 wherein at least one of R<sub>3</sub>, R<sub>4</sub> and R<sub>5</sub> is alkyl.
9. The element of claim 1 wherein two of R<sub>3</sub>, R<sub>4</sub> and R<sub>5</sub> are joined to form an aliphatic ring.
10. The element of claim 1 wherein the substituents X<sub>1</sub>, X<sub>2</sub>, Y, G<sub>1</sub>, and G<sub>2</sub> are individually selected from the group consisting of chloride, fluoride, cyano, acylamino, sulfamoyl, carbamoyl, alkoxy carbonyl, and alkylsulfonyl and in the case of X<sub>1</sub>, X<sub>2</sub> and Y, hydrogen.
11. The element of claim 1 wherein the sum of the pi values for the substituents Z and R<sub>1</sub> is at least 2.5.
12. The element of claim 1 additionally comprising a layer of magnetic particles.
13. The element of claim 12 additionally comprising a yellow colored dye forming masking coupler.
14. A photographic element comprising a support bearing at least one silver halide emulsion layer having associated therewith a 5-pyrazolone photographic coupler represented by the formula:



wherein

- a) substituents X<sub>1</sub>, X<sub>2</sub>, Y, G<sub>1</sub>, and G<sub>2</sub> are individually selected from the group consisting of halogen, alkyl, alkoxy, aryloxy, acylamino, alkylthio, arylthio, sulfonamido, sulfamoyl, sulfamido, carbamoyl, diacylamino, alkoxy carbonyl, aryloxy carbonyl, alkoxy sulfonyl, aryloxy sulfonyl, alkyl sulfonyl, alkylsulfoxyl, arylsulfoxyl, arylsulfonyl, alkoxy carbonylamino, aryloxy carbonylamino, alkylureido, arylureido, acyloxy, nitro, cyano, trifluoromethyl and carboxy and, in the case of X<sub>1</sub>, X<sub>2</sub> and Y, hydrogen;
- b) a, b, and c are individually integers from 0 to 3 provided that "a" cannot be an integer which, combined with the selection of X<sub>1</sub> and X<sub>2</sub>, allows the number of chloride substituents on the ring containing G<sub>1</sub> to exceed 3;
- c) R<sub>1</sub> is selected from the group consisting of G<sub>1</sub> and hydroxyl;
- d) Z is an amine group of the formula:



wherein R<sub>2</sub> is selected from the group consisting of hydrogen, alkyl, alkenyl, aryl, acyl, and heterocyclic; A is carbon and d is 1;

B is comprised of

- (1) an atom of oxygen, nitrogen, sulfur, or carbon bonded to A, said atom also bonded to
- (2) a substituent selected from the group consisting of alkyl, aryl, and heterocyclic groups, wherein, when said atom bonded to A is carbon, B has the formula:



wherein R<sub>3</sub>, R<sub>4</sub>, and R<sub>5</sub> are individually selected from the group consisting of hydrogen, halogen, alkyl, aryl, heterocyclic group and W, wherein W is selected from the group consisting of —OR<sub>6</sub>, —SR<sub>6</sub>, and —NR<sub>7</sub>R<sub>8</sub>, wherein R<sub>6</sub> is selected from the group consisting of alkyl, aryl, and heterocyclic groups, and R<sub>7</sub> and R<sub>8</sub> are individually selected from the group consisting of hydrogen, alkyl, aryl, acyl, alkylsulfonyl, arylsulfonyl and heterocyclic group, provided that, when A is carbon, at least one of R<sub>3</sub>, R<sub>4</sub>, and R<sub>5</sub> is not hydrogen or alkyl and provided that two of R<sub>3</sub>, R<sub>4</sub>, and R<sub>5</sub> may join to form an aliphatic, aromatic, or heterocyclic ring; and

e) the sum of the sigma values for X<sub>1</sub>, X<sub>2</sub>, G<sub>1</sub>, G<sub>2</sub>, and Y is at least 1.3.

\* \* \* \* \*